# EUROPEAN PATENT SPECIFICATION

(11) **EP 0 952 495 B1**
(45) Date of publication and mention of the grant of the patent: **14.01.2009**
(21) Application number: 97909708.6
(22) Date of filing: 31.10.1997
(51) Int. Cl.: G03G 9/093

(54) **ENCAPSULATED TONER AND ITS PRODUCTION PROCESS**
KAPSELTONER UND VERFAHREN ZU DESSEN HERSTELLUNG
TONER ENCAPSULE ET SON PROCEDE DE PRODUCTION

(30) Priority: 06.11.1996 JP 31009196
(43) Date of publication of application: 27.10.1999
(73) Proprietor: Zeon Corporation, Chiyoda-ku Tokyo 100 (JP)
(72) Inventor: OGAWA, Tokudai, Res. & Dev. Center, Kawasaki-ku, Kawasaki-shi, Kanagawa 210 (JP); YANAGIDA, Noboru, Res. & Dev. Center, Kawasaki-ku, Kawasaki-shi, Kanagawa 210 (JP)
(74) Representative: Jones, Helen M.M.
(86) International application number: PCT/JP1997/003972
(87) International publication number: WO 1998/020396

(56) References cited:
- EP-A- 0 615 167
- EP-A- 0 743 564
- GB-A- 2 097 947
- GB-A- 2 109 572
- JP-A- 4 342 264
- JP-A- 53 143 326
- JP-A- 54 094 035

## Description

### <TECHNICAL FIELD>

The present invention relates to a polymerized toner and a production process thereof, and more particularly to a polymerized toner suitable for use in developing an electrostatic latent image formed by an electrophotographic process, electrostatic recording process or the like, and a production process thereof. The present invention also relates to an image forming process comprising using such a polymerized toner, and its use in an image forming apparatus.

### <BACKGROUND ART>

In the electrophotographic process or electrostatic recording process, two-component developers composed of a toner and carrier particles, and one-component developers composed substantially of a toner alone and making no use of any carrier particles are known as developers for making electrostatic latent images visible. The one-component developers include magnetic one-component developers containing magnetic powder, and non-magnetic one-component developers containing no magnetic powder. In the non-magnetic one-component developers, a flowability improver such as colloidal silica is often added independently in order to enhance the flowability of the toner. As the toner, there are generally used colored particles obtained by dispersing a colorant such as carbon black and other additives in a binder resin and granulating the dispersion.

Processes for producing a toner are roughly divided into a grinding process and a polymerization process. In the grinding process, a synthetic resin, a colorant and optional other additives are melted and mixed, the mixture is ground, and the ground product is then classified so as to obtain particles having a desired particle diameter, thereby obtaining a toner. In the polymerization process, a polymerizable monomer composition is prepared by uniformly dissolving or dispersing a colorant, a polymerization initiator and optional various additives such as a crosslinking agent and a charge control agent in a polymerizable monomer, the polymerizable monomer composition is dispersed in an aqueous dispersion medium containing a dispersion stabilizer by means of a stirrer to form minute droplets of the polymerizable monomer composition, and the dispersion containing the minute droplets is then heated to subject the droplets to suspension polymerization, thereby obtaining a toner (polymerized toner) having a desired particle diameter.

In either developer, an electrostatic latent image is actually developed with the toner. In an image forming apparatus such as an electrophotographic apparatus or electrostatic recording apparatus, an electrostatic latent image is generally formed on a photosensitive member evenly charged by exposure to a light pattern, and a toner is applied to the electrostatic latent image to form a toner image (make the latent image visible). The toner image is transferred to a transfer medium such as transfer paper, and the unfixed toner image is then fixed to the transfer medium by a method such as heating, pressing or use of solvent vapor. In the fixing step, the toner is often fusion-bonded to the transfer medium by passing the transfer medium, to which the toner image has been transferred, through between a heating roll (fixing roll) and a press roll to press-bond the toner to the transfer medium under heat.

Images formed by an image forming apparatus such as an electrophotographic copying machine are required to improve their definition year by year. As a toner used in the image forming apparatus, a toner obtained by the grinding process has heretofore been mainly used. The grinding process tends to form colored particles having a wide particle diameter distribution. In order for the toner to exhibit satisfactory developing characteristics, therefore, the ground product must be classified to adjust the particles so as to have a particle diameter distribution limited to a certain extent. However, the classification itself is complicated, and its yield is poor, and so the percent yield of the toner is reduced to a great extent. Therefore, the polymerized toner easy to control its particle diameter without conducting complicated production steps such as classification has come to attract attention in recent years. According to the suspension polymerization process, a polymerized toner having desired particle diameter and particle diameter distribution can be obtained without need of grinding and classification. However, the conventional polymerized toners have involved a problem that they cannot fully meet requirements in recent years, such as the speeding-up of copying, the formation of full-color images and energy saving.

In recent years, copying machines, printers and the like of an electrophotographic system have been required not only to reduce demand power, but also to achieve the speeding-up of copying or printing. A step in which energy is particularly demanded in the electrophotographic system is a fixing step conducted after transferring a toner from a photosensitive member to a transfer medium such as transfer paper. In the fixing step, the toner is fixed to the transfer medium by heating and melting it. Therefore, a heating roll heated to a temperature of at least 150°C is used, and electric power is used as an energy source therefor. There is a demand for lowering the temperature of the heating roll from the viewpoint of energy saving. In order to lower the temperature of the heating roll, it is necessary to use a toner capable of fixing at a temperature lower than that heretofore used. Namely, it is necessary to lower the fixing temperature of the toner itself. The use of the toner capable of fixing at a temperature lower than that heretofore used permits lowering the temperature of the heating roll, and on the other hand shortening the fixing time when the temperature of the heating roll is not very lowered. Therefore, such a toner can meet the speeding-up of copying and the like.

In order to meet requirements, such as energy saving and the speeding-up of copying, from the image forming apparatus in the design of a toner, it is only necessary to lower the glass transition temperature of a binder resin making up the toner. When a toner is made up of a binder resin having a low glass transition temperature, however, the toner becomes poor in the so-called shelf stability because particles themselves of the toner tend to undergo blocking during storage or shipment, or in a toner box of an image forming apparatus, to aggregate.

In recent years, there has been a demand for formation of bright images in color copying or color printing by the electrophotographic system. For example, in the full-color copying, the mere melting and softening of toners in a fixing step to fusion-bond the toners to a transfer medium are not enough, but it is necessary to uniformly melt and mix the toners of different colors to mix their colors. In particular, since color images have come to be often used in OHP (overhead projector) sheets for presentations in various meetings or conferences, toner images fixed to such OHP sheets have been required to permit the formation of bright or clear images on a screen by permeating the sheets, i.e. have excellent permeating the sheets, i.e. have excellent permeability through OHP. In order to meet the excellent permeability through OHP, it is necessary for the toners to uniformly melt on a transparent OHP sheet made of a synthetic resin. Therefore, the melt viscosity of each toner at about the fixing temperature thereof must be designed low compared with the conventional toners. Means for lowering the melt viscosity of the toner include a method in which the molecular weight or glass transition temperature of a binder resin used is lowered compared with the binder resins for the conventional toners. In either method, however, the toner becomes poor in shelf stability because the toner tends to undergo blocking.

EP-A-0615167 describes a method for producing encapsulated toner for heat-and-pressure fixing which comprises a heat fusible core material containing at least a thermoplastic resin and a colouring agent and a shell formed thereon to cover the surface of the core material. The method involves coating the surface of the core material with a hydrophilic shell-forming material to form precursor particles which are then polymerized in the presence of a vinyl polymerizable monomer and an initiator. The polymer used to produce the shell preferably has a glass transition temperature of between 50 and 80°C.

GB-A-2097947 relates to an electrographic toner material. The material comprises encapsulated toner particles which comprise a pressure fixable adhesive core material containing a colourant and a pressure rupturable shell enclosing the core material. The shell is made of a material selected from polyurethane, polyurea and polythiourethane. In all of the examples, encapsulated toner particles with a core comprising carbon black and dibutylphthalate or tricresyl phosphate are illustrated.

GB-A-2109572 describes a toner for development of electrostatic images. The toner detailed comprises a fluid core material selected from the group consisting of (a) fluid substances hardenable under an oxygen-containing atmosphere which may optionally be admixed with a wax and (b) mixtures comprising at least one liquid substance and at least one wax encapsulated within a capsule comprising a vinyl type resin.

As a method for obtaining a polymerized toner having excellent fixing ability, it has theretofore been proposed in, for example, Japanese Patent Application Laid-Open No. 136065/1991 to subject a polymerizable monomer containing a colorant and a charge control agent to suspension polymerization in the presence of a macromonomer. The macromonomer is a relatively long-chain linear molecule having a polymerizable functional group, for example, a group containing an unsaturated bond such as a carbon-carbon double bond, at its molecule chain terminal. According to this method, the macromonomer is incorporated as a monomer unit into the molecular chain of a polymer formed. Therefore, many branches attributable to the long-chain linear molecule of the macromonomer are generated in the molecular chain of the polymer. The polymer apparently becomes a high molecular weight polymer due to entanglement of the branches, i.e., the so-called physical crosslinking, so that the offset resistance of the toner is improved. On the other hand, the physical crosslinking by the macromonomer component is different from chemical crosslinking using a crosslinking monomer such as divinylbenzene and is of a loose crosslinked structure, and so the crosslinked structure is easy to be broken by heating. Accordingly, this polymerized toner is easily melted upon fixing using a heating roll and hence has excellent fixing ability. However, the polymerized toner tends to undergo aggregation among toner particles during storage, and is hence unsatisfactory from the viewpoint of shelf stability.

According to the conventional methods for lowering the fixing temperature of a toner and improving the uniformly melting ability thereof, as described above, an adverse correlation that the fixing ability of the resulting toner is improved, but its shelf stability is lowered arises. As a means for solving this adverse correlation, there has been proposed the so-called capsule type toner in which a toner made up of a binder resin having a low glass transition temperature is covered with a polymer having a high glass transition temperature, thereby improving the blocking resistance of the toner to solve the problem of shelf stability.

As a production process of the capsule type toner, for example, Japanese Patent Application Laid-Open No. 173552/1985 has proposed a process in which a coating layer composed of a colorant, magnetic particles or a conductive agent, and a binder resin is formed on each surface of spherical core particles having a minute particle size by means of a jet mill. As the core particles, there are used particles formed of a thermoplastic transparent resin such as an acrylate resin or styrene resin. In this publication, it has been reported that according to this process, a toner of multilayer structure, which has excellent flowability and improved functional characteristics, can be obtained. When core particles having a low glass transition temperature are used in this method, however, the core particles themselves tend to undergo aggregation. In addition, according to this method, the coating thickness of the binder resin is liable to thicken. Accordingly, this method is difficult to provide a toner improved in both fixing ability and uniformly melting ability while retaining its good shelf stability.

Japanese Patent Application Laid-Open No. 259657/1990 has proposed a process for producing a toner for electrophotography, in which crosslinked toner particles prepared by suspension polymerization are added to a solution with an encapsulating polymer, a charge control agent and a parting agent dissolved in an organic solvent, and a poor solvent is then added to the resultant mixture to form a coating film of the encapsulating polymer containing the charge control agent and parting agent on each surface of the crosslinked toner particles. According to this process, however, it is difficult to obtain spherical particles because the solubility of the encapsulating polymer is reduced by the addition of the poor solvent to deposit the polymer on each surface of the crosslinked toner particles. The capsule wall formed on the surface of each crosslinked toner particle according to this process is uneven in thickness, and moreover is relatively thick. As a result, the effects of improving development properties and fixing ability become insufficient.

Japanese Patent Application Laid-Open No. 45558/1982 has proposed a process for producing a toner for developing electrostatic latent images, in which core particles formed by polymerization are mixed with and dispersed in a 1 to 40 wt.% aqueous latex solution, and a water-soluble inorganic salt is then added to the dispersion to form a coating layer formed of fine particles obtained by emulsion polymerization on each surface of the core particles. However, this process has involved a drawback that the temperature and humidity dependence of charge properties of the resultant toner becomes great due to the influence of a surfactant and the inorganic salt remaining on the fine particles, and the charge properties are deteriorated under high-temperature and high-humidity conditions in particular.

Japanese Patent Application Laid-Open No. 118758/1986 discloses a process for producing a toner, in which a composition containing a vinyl monomer, a polymerization initiator and a colorant is subjected to suspension polymerization to obtain core particles, and another vinyl monomer capable of providing a polymer having hydrophilicity at least equal to that of the resin contained in the core particles and a glass transition temperature higher than that of said resin is polymerized in the presence of the core particles to form shell on each of the core particles. This publication also discloses that a parting agent such as low molecular weight polyethylene, carnauba wax or silicone oil may be added to the core particles for preventing a part of the toner melted from adhering to the surface of a fixing roll. According to this process, however, the vinyl monomer for forming the shell is caused to be adsorbed on each of the core particles to grow it, so that in many cases, it may be difficult to create a clear core-shell structure because the vinyl monomer absorbed in the interior of the core particles is polymerized. Accordingly, this process is difficult to provide a toner sufficiently improved in shelf stability. In addition, in order to create a clear core-shell structure so as to improve the shelf stability, it has been necessary to thicken the thickness of the shell.

Japanese Patent Application Laid-Open No. 128908/1995 discloses a process for directly producing a polymerized toner by subjecting a monomer composition containing a polymerizable monomer, a colorant and a parting agent to suspension polymerization in an aqueous medium, the process comprising the steps of causing the parting agent to contain in a proportion of 10 to 40 parts by weight per 100 parts by weight of the polymerizable monomer and removing the parting agent on the surface of the toner formed after completion of the polymerization step. According to this process, when a polymer having a polar group is added to the monomer to polymerize the monomer, a core-shell structure is formed because the polar polymer gathers on each surface layer of polymer particles formed. In addition, the parting agent on the surface of the toner is removed, so that staining due to attachment of the parting agent (wax) to a developing drum, a photosensitive drum, a transfer drum and/or the like can be reduced. However, this process cannot fully improve the shelf stability, fixing temperature and the like of the toner and tends to cause fogging, deterioration of image density, etc.

### <DISCLOSURE OF THE INVENTION>

It is an object of the present invention to provide a polymerized toner which has a low fixing temperature and uniformly melting ability, and is excellent in shelf stability (blocking resistance) and hard to cause fogging, deterioration of image density, etc., and a production process thereof.

Another object of the present invention is to provide a polymerized toner which can meet the speeding-up of copying or printing, the formation of full-color images, and energy saving, and a production process thereof.

A further object of the present invention is to provide a polymerized toner capable of forming a toner image which exhibits excellent permeability (permeability through OHP) when conducting printing on an OHP sheet with the toner and fixing the resulting image thereto, and a production process thereof.

A still further object of the present invention is to provide an image forming process comprising using the polymerized toner having such excellent various properties, and an image forming apparatus in which said polymerized toner is contained.

The present inventors have carried out an extensive investigation with a view toward overcoming the above-described problems involved in the prior art. As a result, the inventors have conceived of a polymerized toner of core-shell structure as defined in claim 1.

According to the polymerized toner of the present invention, the core particles containing the polyfunctional ester compound and the polymer component having a lower glass transition temperature permit lowering the fixing temperature of the toner, also improving the uniformly melting ability, meeting requirements such as the speeding-up of copying or printing, the formation of full-color images and good permeability through OHP, and further forming a high-quality image because they make it hard to cause fogging, deterioration of image density and the like. On one hand, according to the polymerized toner of the present invention, each of the core particles can be covered with the thin shell, so that the toner can exhibit good shelf stability (blocking resistance) and moreover fully meet various requirements such as fixing ability and uniformly melting ability.

The present invention has been led to completion on the basis of these findings.

According to the present invention, there is also provided process for producing a polymerized toner of the core-shell structure, as defined in claim 7.

According to the present invention, there is further provided an image forming process as claimed in claim 25.

According to the present invention, there is still further provided a use of such a polymerized toner in an image forming apparatus according to claim 26, comprising a photosensitive member, a means for charging the surface of the photosensitive member, a means for forming an electrostatic latent image on the surface of the photosensitive member, a means for receiving a toner, a means for supplying the toner to develop the electrostatic latent image on the surface of the photosensitive member, thereby forming a toner image, and a means for transferring the toner image from the surface of the photosensitive member to a transfer medium, wherein the means for receiving the toner contains the above-described polymerized toner of core-shell structure.

### <BRIEF DESCRIPTION OF THE DRAWING>

FIG. 1 is a cross-sectional view illustrating an example of an image forming apparatus to which a polymerized toner according to the present invention is applied.

### <BEST MODE FOR CARRYING OUT THE INVENTION>

The polymerized toner according to the present invention is a polymerized toner of a core-shell structure, comprising core particles and shell which covers each of the core particles. The polymerized toner according to the present invention can be produced by polymerizing a polymerizable monomer for shell in the presence of core particles. The core particles comprise, as essential components, a polyfunctional ester compound formed of a trifunctional or still higher polyfunctional polyhydric alcohol and a carboxylic acid having 10 to 30 carbon atoms and a colorant in a polymer component (binder resin). The glass transition temperature of a polymer component making up the shell is higher than that of the polymer component making up the core particles.

### Polyfunctional ester compound:

The polyfunctional ester compound useful in the practice of the present invention is an ester formed of a trifunctional or still higher polyfunctional polyhydric alcohol and a carboxylic acid.

Examples of the trifunctional or still higher polyfunctional polyhydric alcohol include aliphatic alcohols such as glycerol, pentaerythritol and pentaglycerol; alicyclic alcohols such as phloroglucitol, quercitol and inositol; aromatic alcohols such as tris-(hydroxymethyl)benzene; saccharides such as D-erythrose, L-arabinose, D-mannose, D-galactose, D-fructose, L-rhamnose, saccharose, maltose and lactose; and sugar alcohols such as erythoritol, D-threitol, L-arabitol, adonitol and xylitol. Of these, pentaerythritol is preferred.

Examples of the carboxylic acid include aliphatic carboxylic acids such as acetic acid, butyric acid, caproic acid, enanthic acid, caprylic acid, pelargonic acid, capric acid, undecanoic acid, lauric acid, myristic acid, stearic acid, margaric acid, arachidic acid, cerotic acid, melissic acid, erucic acid, brassidic acid, sorbic acid, linolic acid, linolenic acid, behenolic acid, tetrolic acid and ximenynic acid; alicyclic carboxylic acids such as cyclohexanecarboxylic acid, hexahydro-isophthalic acid, hexahydroterephthalic acid and 3,4,5,6-tetrahydrophthalic acid; and aromatic carboxylic acids such as benzoic acid, toluic acid, cuminic acid, phthalic acid, isophthalic acid, terephthalic acid, trimesic acid, trimellitic acid and hemimellitic acid. Of these, carboxylic acids having 10 to 30 carbon atoms are used, preferably, 13 to 25 carbon atoms, and aliphatic carboxylic acids having the said number of carbon atoms are more preferred. Among the aliphatic carboxylic acids, stearic acid and myristic acid are particularly preferred.

In the polyfunctional ester compound used in the present invention, the carboxylic acids reacting with at least 3 functional groups (OH groups) of the polyhydric alcohol to form respective ester bonds may be the same or different from one another. When the kinds of the carboxylic acids reacting with the polyhydric alcohol are different from one another, it is desirable that a difference between the maximum value and the minimum value in the number of carbon atoms among the carboxylic acids be preferably at most 9, more preferably at most 5.

The polyfunctional ester compound is preferably a compound represented by the formula (I): wherein R¹, R², R³ and R⁴ are independently an alkyl group or phenyl group, and the number of carbon atoms of the alkyl group or phenyl group is 10 to 30, preferably 13 to 25.

As specific examples of the polyfunctional ester compound, may be mentioned pentaerythritol tetrastearate [a compound in which R¹, R², R³ and R⁴ in the formula (I) are all CH₃(CH₂)₁₆ groups], pentaerythritol tetramyristate [a compound in which R¹, R², R³ and R⁴ in the formula (I) are all CH₃(CH₂)₁₂ groups] and glycerol triarachidate. The polyfunctional ester compound is preferably easily soluble in a polymerizable monomer for core.

The polyfunctional ester compound is used in a proportion of generally 0.1 to 40 parts by weight, preferably 1 to 20 parts by weight, more preferably 3 to 15 parts by weight per 100 parts by weight of a polymer component making up core particles or a monomer for forming the polymer component (polymerizable monomer for core). The proportion of the polyfunctional ester compound used falls within the above range, whereby a polymerized toner, which has a low fixing temperature and uniformly melting ability, and is excellent in shelf stability (blocking resistance) and hard to cause fogging, deterioration of image density, etc., can be provided. If the proportion of the polyfunctional ester compound used is too low, its effect becomes little. If the proportion is too high on the other hand, it is difficult to form the core particles, and the shelf stability of the resulting polymerized toner is also deteriorated.

### Colorant:

As examples of the colorant useful in the practice of the present invention, may be mentioned dyes and pigment such as carbon black, titanium white, Nigrosine Base, aniline blue, Chalcoil Blue, chrome yellow, ultramarine blue, Orient Oil Red, Phthalocyanine Blue and Malachite Green oxalate; and magnetic powders such as cobalt, nickel, diiron trioxide, triiron tetroxide, manganese iron oxide, zinc iron oxide and nickel iron oxide.

Examples of colorants for magnetic color toners include C.I. Direct Red 1, C.I. Direct Red 4, C.I. Acid Red 1, C.I. Basic Red 1, C.I. Mordant Red 30, C.I. Direct Blue 1, C.I. Direct Blue 2, C.I. Acid Blue 9, C.I. Acid Blue 15, C.I. Basic Blue 3, C.I. Basic Blue 5, C.I. Mordant Blue 7, C.I. Direct Green 6, C.I. Basic Green 4 and C.I. Basic Green 6. Examples of pigments for magnetic color toners include chrome yellow, cadmium yellow, Mineral Fast Yellow, Navel Yellow, Naphthol Yellow S, Hansa Yellow G, Permanent Yellow NCG, Tartrazine Lake, chrome orange, molybdenum orange, Permanent Orange GTR, Pyrazolone Orange, Benzidine Orange, cadmium red, Permanent Red 4R, Watchung Red Ca, eosine lake, Brilliant Carmine 3B, manganese violet, Fast Violet B, Methyl Violet Lake, iron blue, cobalt blue, Alkali Blue Lake, Victoria Blue Lake, Phthalocyanine Blue, Fast Sky Blue, Indanthrene Blue BC, chrome green, chromium oxide, Pigment Green B, Malachite Green Lake and Final Yellow Green G.

Examples of magenta color pigments for full-color toners include C.I. Pigment Red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48, 49, 50, 51, 52, 53, 54, 55, 57, 58, 60, 63, 64, 68, 81, 83, 87, 88, 89, 90, 112, 114, 122, 123, 163, 202, 206, 207 and 209; C.I. Pigment Violet 19; and C.I. Vat Red 1, 2, 10, 13, 15, 23, 29 and 35.

Examples of magenta dyes for full-color toners include oil-soluble dyes such as C.I. Solvent Red 1, 3, 8, 23, 24, 25, 27, 30, 49, 81, 82, 83, 84, 100, 109 and 121; C.I. Disperse Red 9; C.I. Solvent Violet 8, 13, 14, 21 and 27; and C.I. Disperse Violet 1; and basic dyes such as C.I. Basic Red 1, 2, 9, 12, 13, 14, 15, 17, 18, 22, 23, 24, 27, 29, 32, 34, 35, 36, 37, 38, 39 and 40; and C.I. Basic Violet 1, 3, 7, 10, 14, 15, 21, 25, 26, 27 and 28.

Examples of cyan color pigments for full-color toners include C.I. Pigment Blue 2, 3, 15, 16 and 17; C.I. Vat Blue 6; C.I. Acid Blue 45; and copper phthalocyanine dyes with 1 to 5 phthalimidomethyl groups added to a phthalocyanine skeleton.

Examples of yellow color pigments for full-color toners include C.I. Pigment Yellow 1, 2, 3, 4, 5, 6, 7, 10, 11, 12, 13, 14, 15, 16, 17, 23, 65, 73, 83 and 138; and C.I. Vat Yellow 1, 3 and 20.

These dyes or pigments are used in a proportion of generally 0.1 to 20 parts by weight, preferably 1 to 10 parts by weight per 100 parts by weight of the polymer component making up the core particles or the polymerizable monomer for core. The magnetic powder is used in a proportion of generally 1 to 100 parts by weight, preferably 5 to 50 parts by weight per 100 parts by weight of the polymer component making up the core particles or the polymerizable monomer for core.

### Core particles :

The core particles useful in the practice of the present invention comprise, as a polymer component (binder resin), a (co)polymer of a vinyl monomer, such as a polyester resin, or a (meth)acrylic ester-styrene copolymer. As the polymer component for the core particles, the (meth)acrylic ester-styrene copolymer is preferred because it is easy to form particles by polymerization and control the glass transition temperature of the polymer component.

In the polymerized toner according to the present invention, the volume average particle diameter (dv) of the core particles is generally 0.5 to 20 µm, preferably 1 to 10 µm. If the core particles are too great, the resolution of an image formed with such a toner tends to lower. The ratio (dv)/(dp) of the volume average particle diameter (dv) to a number average particle diameter (dp) in the core particles is generally at most 1.7, preferably at most 1.5. If this ratio is too high, the resolution of an image formed with such a toner tends to lower.

No particular limitation is imposed on the production process of the core particles used in the present invention, and any of emulsion polymerization, suspension polymerization, precipitation polymerization and soap-free polymerization may be used. However, a process comprising subjecting a polymerizable monomer for core to suspension polymerization is preferred in that the polyfunctional ester compound and colorant can be uniformly contained in each of core particles formed, and the fixing ability of the resulting toner is improved.

The polymerizable monomer for core used in the present invention forms a polymer having a glass transition temperature of generally 80°C or lower, preferably 10 to 70°C, more preferably 15 to 60°C. As the polymerizable monomer for core, there may be used one of such monomers or any combination of such monomers. If the glass transition temperature of a polymer formed of the polymerizable monomer for core is too high, the resulting polymerized toner comes to have a higher fixing temperature and deteriorated permeability through OHP and can not meet the speeding-up of copying or printing.

The glass transition temperature (Tg) of the polymer is a calculated value (referred to as calculated Tg) calculated out according to the kind(s) and proportion(s) of monomer(s) used. When the monomer used is one, the Tg of a homopolymer formed from this monomer is defined as Tg of the polymer in the present invention. For example, the Tg of polystyrene is 100°C. Therefore, when styrene is used as a monomer by itself, the monomer can be said to form a polymer having a Tg of 100°C. When monomers used are two or more, and the polymer formed is a copolymer, the Tg of the copolymer is calculated out according to the kinds and proportions of the monomers used. For example, when 78 wt.% of styrene and 22 wt.% of n-butyl acrylate are used as monomers, the monomers can be said to form a polymer having a Tg of 50°C because the Tg of a styrene-n-butyl acrylate copolymer formed at this monomer ratio is 50°C.

The definition of "a polymerizable monomer for core, which is capable of forming a polymer having a glass transition temperature of 80°C or lower" does not mean that when plural monomers are used, the individual monomers must form respective polymers having a Tg of 80°C or lower. When one monomer is used, the Tg of a homopolymer formed from the monomer must be 80°C or lower. When two or more monomers are used, however, it is only necessary for the Tg of a copolymer formed from the monomer mixture to be 80°C or lower. Therefore, those which separately form a homopolymer having a Tg higher than 80°C may be contained in the monomer mixture. For example, although the Tg of a styrene homopolymer is 100°C, styrene may be used as a component of the polymerizable monomer for core so far as a copolymer having a Tg of 80°C or lower can be formed by using a mixture of styrene with a monomer (for example, n-butyl acrylate) which forms a homopolymer having a low Tg.

In the present invention, vinyl monomers are generally used as the polymerizable monomer for core. Various kinds of vinyl monomers are used either singly or in combination of two or more thereof so as to adjust the Tg of the resulting polymer within the desired range.

Examples of the vinyl monomers used in the present invention include styrenic monomers such as styrene, vinyltoluene and α-methylstyrene; acrylic acid and methacrylic acid; (meth)acrylic acid derivatives such as methyl acrylate, ethyl acrylate, propyl acrylate, butyl acrylate, 2-ethylhexyl acrylate, dimethylaminoethyl acrylate, methyl methacrylate, ethyl methacrylate, propyl methacrylate, butyl methacrylate, 2-ethylhexyl methacrylate, dimethylaminoethyl methacrylate, acrylonitrile, methacrylonitrile, acrylamide and methacrylamide; ethylenically unsaturated monoolefins such as ethylene, propylene and butylene; vinyl halides such as vinyl chloride, vinylidene chloride and vinyl fluoride; vinyl esters such as vinyl acetate and vinyl propionate; vinyl ethers such as vinyl methyl ether and vinyl ethyl ether; vinyl ketones such as vinyl methyl ketone and methyl isopropenyl ketone; and nitrogen-containing vinyl compounds such as 2-vinylpyridine, 4-vinylpyridine and N-vinylpyrrolidone. These vinyl monomers may be used either singly or in any combination thereof. Of these, the styrenic monomers, or the (meth)acrylic acid derivatives are preferably used as a polymerizable monomer for core.

Of these, a combination of a styrenic monomer with a (meth)acrylic acid derivative is preferably used as the polymerizable monomer for core. As particularly preferable specific examples thereof, may be mentioned combinations of styrene with butyl acrylate (i.e., n-butyl acrylate), and styrene with 2-ethylhexyl acrylate.

It is preferred from the viewpoint of improvement in the shelf stability of the resulting polymerized toner to use a crosslinking monomer in combination with the polymerizable monomer for core composed of the vinyl monomer(s). Examples of the crosslinking monomer include aromatic divinyl compounds such as divinylbenzene, divinylnaphthalene and derivatives thereof; diethylenic esters of unsaturated carboxylic acids such as ethylene glycol dimethacrylate and diethylene glycol dimethacrylate; divinyl compounds such as N,N-divinylaniline and divinyl ether; and compounds having at least three vinyl groups.

These crosslinking monomers may be used either singly or in any combination thereof. It is desirable that the crosslinking monomer be used in a proportion of generally 0.1 to 5 parts by weight, preferably 0.3 to 2 parts by weight per 100 parts by weight of the polymerizable monomer for core.

In the present invention, a macromonomer is preferably copolymerized with the polymerizable monomer for core from the viewpoint of improving the balance between the shelf stability and fixing ability of the resulting polymerized toner. In order to copolymerize the macromonomer, it is only necessary to polymerize a polymerizable monomer composition containing the polyfunctional ester compound, the colorant and the polymerizable monomer for core in the presence of the macromonomer to synthesize colored polymer particles (core particles). In fact, it is preferred that the macromonomer be contained in the polymerizable monomer composition to conduct suspension polymerization.

The macromonomer (also referred to as macromer) is a relatively long-chain linear molecule having a polymerizable functional group (for example, a group containing an unsaturated bond such as a carbon-carbon double bond) at its molecular chain terminal. The macromonomer is preferably an oligomer or polymer having a polymerizable vinyl functional group at its molecular chain terminal and a number average molecular weight of generally 1,000 to 30,000. If a macromonomer having a too low number average molecular weight is used, the surface part of the resulting polymerized toner becomes soft, and its shelf stability shows a tendency to deteriorate. If a macromonomer having a too high number average molecular weight is used on the other hand, the flowability of the macromonomer becomes poor, resulting in a polymerized toner deteriorated in fixing ability and shelf stability.

Examples of the polymerizable vinyl functional group which the macromonomer has at its molecular chain terminal include an acryloyl group and a methacryloyl group, with the methacryloyl group being preferred from the viewpoint of easy copolymerization.

The macromonomer used in the present invention preferably has a glass transition temperature higher than that of a polymer obtained by polymerizing the polymerizable monomer for core. A difference in Tg between the polymer obtained by polymerizing the polymerizable monomer for core and the macromonomer may be relative. For example, when the polymerizable monomer for core is such that forms a polymer having a Tg of 80°C, it is only necessary for the macromonomer to have a Tg higher than 80°C. When the polymerizable monomer for core is such that forms a polymer having a Tg of 50°C, the macromonomer may also be that having a Tg of, for example, 60°C. The Tg of the macromonomer is a value measured by means of an ordinary measuring device such as a DSC.

As specific examples of the macromonomer used in the present invention, may be mentioned polymers obtained by polymerizing styrene, styrene derivatives, methacrylic esters, acrylic esters, acrylonitrile and methacrylonitrile either singly or in combination of two or more monomers thereof; macromonomers having a polysiloxane skeleton; and those disclosed in Japanese Patent Application Laid-Open No. 203746/1991, pages 4 to 7.

Of these macromonomers, hydrophilic macromonomers, in particular, polymers obtained by polymerizing methacrylic esters or acrylic esters either singly or in combination of two or more monomers thereof are preferred in the present invention.

The amount of the macromonomer used is generally 0.01 to 10 parts by weight, preferably 0.03 to 5 parts by weight, more preferably 0.05 to 1 part by weight per 100 parts by weight of the polymerizable monomer for core. If the amount of the macromonomer used is too little, the shelf stability of the resulting polymerized toner is deteriorated. If the amount of the macromonomer used is too great, the fixing ability of the resulting polymerized toner is deteriorated.

In the present invention, it is preferred that the core particles be provided by subjecting the polymerizable monomer for core, the macromonomer and optionally the crosslinking monomer to suspension polymerization.

The suspension polymerization is generally performed in an aqueous dispersion medium containing a dispersing agent. More specifically, the suspension polymerization is conducted by mixing a polymerizable monomer (vinyl monomer) for core, a polyfunctional ester compound, a colorant, a macromonomer, an optional crosslinking monomer, a radical polymerization initiator and other additives, uniformly dispersing them by means of a ball mill or the like to prepare a liquid mixture (polymerizable monomer composition), pouring the liquid mixture into an aqueous dispersion medium containing a dispersing agent, dispersing the liquid mixture in the dispersion medium by means of a mixer having high shearing force to form minute droplets, and then subjecting them to suspension polymerization at a temperature of generally 30 to 200°C.

A dispersing agent preferably used in the present invention is colloid of a hardly water-soluble metallic compound. As examples of the hardly water-soluble metallic compound, may be mentioned sulfates such as barium sulfate and calcium sulfate; carbonates such as barium carbonate, calcium carbonate and magnesium carbonate; phosphates such as calcium phosphate; metal oxides such as aluminum oxide and titanium oxide; and metal hydroxides such as aluminum hydroxide, magnesium hydroxide and ferric hydroxide. Of these, colloids of hardly water-soluble metal hydroxides are preferred because the particle diameter distribution of the resulting polymer particles can be narrowed, and the brightness or sharpness of an image formed from such a polymerized toner is enhanced.

The colloid of the hardly water-soluble metal hydroxide is not limited by the production process thereof. However, colloid of a hardly water-soluble metal hydroxide obtained by adjusting the pH of an aqueous solution of a water-soluble polyvalent metallic compound to 7 or higher, in particular, colloid of a hardly water-soluble metal hydroxide formed by reacting a water-soluble polyvalent metallic compound with an alkali metal hydroxide in an aqueous phase is preferred. This colloid is used as an aqueous dispersion.

The colloid of the hardly water-soluble metal hydroxide used in the present invention preferably has number particle diameter distributions, D₅₀ (50% cumulative value of number particle diameter distribution) of at most 0.5 µm and D₉₀ (90% cumulative value of number particle diameter distribution) of at most 1 µm. If the particle diameter of the colloid is too great, the stability of the suspension polymerization is broken, and the shelf stability of the resulting polymerized toner is deteriorated.

The dispersing agent is generally used in a proportion of 0.1 to 20 parts by weight per 100 parts by weight of the monomer for core. If the amount of the dispersing agent used is too little, it is difficult to achieve sufficient polymerization stability, so that the resulting polymer tends to aggregate. If the amount of the dispersing agent used is too great on the other hand, the effect of the dispersing agent on polymerization stability is saturated, which is uneconomical. In addition, the viscosity of the aqueous dispersion medium becomes too high, resulting in difficulty of forming fine droplets of the liquid mixture.

In the present invention, a water-soluble polymer may be used as a dispersing agent as needed. As examples of the water-soluble polymer, may be mentioned polyvinyl alcohol, methyl cellulose and gelatin. In the present invention, there is no need to use any surfactant. However, a surfactant may be used for the purpose of stably conducting the suspension polymerization so far as the dependence of the charge properties of the resulting polymerized toner on environment does not become large.

As examples of the radical polymerization initiator, may be mentioned water-soluble polymerization initiators, such as persulfates such as potassium persulfate and ammonium persulfate; and azo compounds such as 4,4-azobis(4-cyanovaleric acid), 2,2-azobis(2-amidinopropane) bihydrochloride, 2,2-azobis-2-methyl-N-1,1-bis-(hydroxymethyl)-2-hydroxyethylpropionamide, 2,2'-azobis-(2,4-dimethylvaleronitrile), 2,2'-azobisisobutyronitrile and 1,1'-azobis(1-cyclohexanecarbonitrile); and oil-soluble polymerization initiators, such as peroxides such as methyl ethyl peroxide, di-t-butyl peroxide, acetyl peroxide, dicumyl peroxide, lauroyl peroxide, benzoyl peroxide, t-butyl peroxy-2-ethylhexanoate, di-isopropyl peroxydicarbonate and di-t-butyl peroxyisophthalate. Redox initiators composed of combinations of these polymerization initiators with a reducing agent may also be mentioned.

Of these radical polymerization initiators, the oil-soluble radical initiators are preferred, with oil-soluble radical initiators selected from among organic peroxides whose ten-hour half-life temperatures are 60 to 80°C, preferably 65 to 80°C and whose molecular weights are 250 or lower being particularly preferred. Of the oil-soluble radical initiators, t-butyl peroxy-2-ethyl-hexanoate is particularly preferred because the resulting polymerized toner scarcely gives odor upon printing and barely causes environmental destruction by volatile components such as odor.

The amount of the polymerization initiator used is generally 0.001 to 3 wt.% based on the aqueous medium. If the amount of the polymerization initiator used is less than 0.001 wt.%, the rate of polymerization becomes slow. If the amount exceeds 3 wt.%, particles having a particle diameter smaller than 1 µm are formed as a by-product. It is hence not preferable to use the initiator in such a little or great amount.

In the present invention, as needed, various kinds of additives such as a molecular weight modifier may be used by mixing them with the polymerizable monomer for core.

Examples of the molecular weight modifier include mercaptans such as t-dodecylmercaptan, n-dodecylmercaptan and n-octylmercaptan; and halogenated hydrocarbons such as carbon tetrachloride and carbon tetrabromide. The molecular weight modifier may be added before the initiation of the polymerization or in the course of the polymerization. The molecular weight modifier is used in a proportion of generally 0.01 to 10 parts by weight, preferably 0.1 to 5 parts by weight per 100 part by weight of the polymerizable monomer for core.

In the polymerized toner according to the present invention, the polyfunctional ester compound also fulfills a function as a parting agent, and so it is not always necessary to use any other parting agent. However, a parting agent, for example, a low molecular weight polyolefin such as low molecular weight polyethylene, low molecular weight polypropylene or low molecular weight polybutylene; or a paraffin wax, may be used within limits not impeding the objects of the present invention.

A lubricant such as oleic acid or stearic acid; a dispersion aid such as a silane or titanium coupling agent; and/or the like may also be used with a view toward uniformly dispersing the colorant in the core particles. Such a lubricant or dispersion aid is generally used in a proportion of about 1/1,000 to 1/1 based on the weight of the colorant.

The polymerization for obtaining the core particles is continued until the conversion of the polymerizable monomer into a polymer reaches generally at least 80%, preferably at least 85%, more preferably at least 90%. If the conversion into the polymer is lower than 80%, a great amount of the polymerizable monomer for core remains unreacted, so that each surface of the resultant core particles is covered with a copolymer of the polymerizable monomer for core and a polymerizable monomer for shell even when the polymerizable monomer for shell is added to conduct polymerization. Therefore, a difference in Tg between the core particles and the shell becomes small, and so the shelf stability of the resulting polymerized toner tends to lower.

### Shell:

In the present invention, the polymerized toner can be obtained by polymerizing a polymerizable monomer for shell in the presence of the core particles.

The polymerizable monomer for shell used in the present invention is such that can form a polymer having a glass transition temperature higher than that of the polymer component making up the core particles. A difference in Tg between the polymer obtained by the polymerizable monomer for shell and the polymer component making up the core particles is relative.

As the polymerizable monomer for shell, there are be used monomers capable of forming a polymer having a glass transition temperature higher than 80°C, for example, styrene and methyl methacrylate, either singly or in combination of two or more monomers thereof. However, the glass transition temperature of the polymer formed from the polymerizable monomer for shell must be preset so as to be higher than the glass transition temperature of the polymer component of the core particles. In order to improve the shelf stability of the resulting polymerized toner, the glass transition temperature of the polymer formed from the polymerizable monomer for shell is preset within a range of 80 to 110°C. If the glass transition temperature of the polymer formed from the polymerizable monomer for shell is too low, the shelf stability of the resulting polymerized toner may be lowered in some cases even if such a glass transition temperature is higher than that of the polymer component of the core particles. In many cases, the glass transition temperature of the polymer component of the core particles may be represented by the calculated Tg of a polymer formed from the polymerizable monomer for core.

A difference in glass transition temperature between the polymer formed from the polymerizable monomer for core and the polymer formed from the polymerizable monomer for shell is at least 10°C, preferably at least 20°C, more preferably at least 30°C.

The polymerizable monomer for shell is preferably polymerized in the presence of the core particles after it is formed into droplets smaller than the number average particle diameter of the core particles in an aqueous dispersion medium. If the droplet diameter of the droplets of the polymerizable monomer for shell is too great, the shelf stability of the resulting polymerized toner shows a tendency to lower.

In order to form the polymerizable monomer for shell into fine droplets, a mixture of the polymerizable monomer for shell and the aqueous dispersion medium is subjected to a finely dispersing treatment by means of, for example, an ultrasonic emulsifier. It is preferred that the aqueous dispersion thus obtained be added to the reaction system in which the core particles are present.

The polymerizable monomer for shell is not particularly limited by solubility in water at 20°C. However, a polymerizable monomer for shell having a high solubility in water, specifically, a monomer having a solubility of at least 0.1 wt.% in water at 20°C becomes liable to quickly migrate to the surfaces of the core particles, so that a polymerized toner having good shelf stability is easy to obtain.

On the other hand, when a polymerizable monomer for shell having a solubility lower than 0.1 wt.% in water at 20°C is used, its migration to the surfaces of the core particles becomes slow. Therefore, it is preferable to polymerize such a monomer after adding it in the form of fine droplets to the reaction system. Even when a polymerizable monomer for shell having a solubility lower than 0.1 wt.% in water at 20°C is used, the polymerizable monomer for shell becomes easy to quickly migrate to the surfaces of the core particles when an organic solvent having a solubility of at least 5 wt.% in water at 20°C is added to the reaction system, so that a polymerized toner having good shelf stability is easy to obtain.

Examples of the polymerizable monomer for shell having a solubility lower than 0.1 wt.% in water at 20°C include styrene, butyl acrylate, 2-ethylhexyl acrylate, ethylene and propylene. Examples of the polymerizable monomer for shell having a solubility of at least 0.1 wt.% in water at 20°C include (meth)acrylic esters such as methyl methacrylate and methyl acrylate; amides such as acrylamide and methacrylamide; vinyl cyanide compounds such as acrylonitrile and methacrylonitrile; nitrogen-containing vinyl compounds such as 4-vinylpyridine; and vinyl acetate and acrolein.

As examples of an organic solvent preferably used in the case where the polymerizable monomer for shell having a solubility lower than 0.1 wt.% in water at 20°C is used, may be mentioned lower alcohols such as methanol, ethanol, isopropyl alcohol, n-propyl alcohol and butyl alcohol; ketones such as acetone and methyl ethyl ketone; cyclic ethers such as tetrahydrofuran and dioxane; ethers such as dimethyl ether and diethyl ether; and amides such as dimethylformamide.

The organic solvent is added in such an amount that the solubility of the polymerizable monomer for shell in the dispersion medium (containing water and the organic solvent in combination) is at least 0.1 wt.%. The specific amount of the organic solvent added varies according to the kind of the organic solvent, and the kind and amount of the polymerizable monomer for shell. However, it is generally 0.1 to 50 parts by weight, preferably 0.1 to 40 parts by weight, more preferably 0.1 to 30 parts by weight per 100 parts by weight of the aqueous dispersion medium. No particular limitation is imposed on the order of addition of the organic solvent and the polymerizable monomer for shell to the reaction system. In order to facilitate the migration of the polymerizable monomer for shell to the core particles to make easy to obtain a polymerized toner having good shelf stability, however, it is preferable to first add the organic solvent to the reaction system and then add the polymerizable monomer for shell.

When a monomer having a solubility lower than 0.1 wt.% in water at 20°C and a monomer having a solubility of at least 0.1 wt.% in water at 20°C are used in combination, it is preferable to first add the monomer having a solubility of at least 0.1 wt.% in water at 20°C to polymerize it, then add the organic solvent, and further add the monomer having a solubility lower than 0.1 wt.% in water at 20°C to polymerize it. According to this adding process, the Tg of the polymer obtained from the polymerizable monomer for shell, which is polymerized in the presence of the core particles for the purpose of controlling the fixing temperature of the resulting polymerized toner, and the amount of the monomer added can be suitably controlled.

The polymerizable monomer for shell is preferably used in combination with a charge control agent. The incorporation of the charge control agent into the shell permits improving the charge properties of the resulting polymerized toner. As the charge control agent, there may be used various kinds of charge control agents for positive charge and negative charge. As specific examples of the charge control agents, may be mentioned Nigrosine NO1 (product of Orient Chemical Industries Ltd.), Nigrosine EX (product of Orient Chemical Industries Ltd.), Spiron Black TRH (product of Hodogaya Chemical Co., Ltd.), T-77 (product of Hodogaya Chemical Co., Ltd.), Bontron S-34 (product of Orient Chemical Industries Ltd.) and Bontron E-84 (product of Orient Chemical Industries Ltd.). The charge control agent is used in a proportion of generally 0.01 to 10 parts by weight, preferably 0.1 to 5 parts by weight per 100 parts by weight of the polymerizable monomer for core.

As examples of a specific process for polymerizing the polymerizable monomer for shell in the presence of the core particles, may be mentioned a process in which the polymerizable monomer for shell is added to the reaction system of the polymerization reaction which has been conducted for obtaining the core particles, thereby continuously conducting polymerization, and a process in which the core particles obtained in a separate reaction system are charged, to which the polymerizable monomer for shell is added, thereby conducting polymerization stepwise.

The polymerizable monomer for shell may be added to the reaction system in one lot, or continuously or intermittently by means of a pump such as a plunger pump.

In order to make easy to obtain polymer particles of core-shell structure, it is preferable to add a water-soluble radical initiator at the time the polymerizable monomer for shell is added. It is considered that when the water-soluble radical initiator is added upon the addition of the polymerizable monomer for shell, the water-soluble initiator enters in the vicinity of each outer surface of the core particles to which the polymerizable monomer for shell has migrated, so that a polymer layer (shell) is easy to form on the core particle surface.

As examples of the water-soluble radical initiator, may be mentioned persulfates such as potassium persulfate and ammonium persulfate; azo initiators such as 4,4-azo-bis(4-cyanovaleric acid), 2,2-azobis(2-amidinopropane) bihydrochloride and 2,2-azobis-2-methyl-N-1,1-bis-(hydroxymethyl)-2-hydroxyethylpropionamide; and combinations of an oil-soluble initiator such as cumene peroxide with a redox catalyst. The amount of the water-soluble radical initiator used is generally 0.001 to 1 wt.% based on the aqueous medium.

### Polymerized toner:

In the polymerized toner according to the present invention, a weight ratio of the polymerizable monomer for core to the polymerizable monomer for shell is generally 40/60 to 99.9/0.1, preferably 60/40 to 99.5/0.5, more preferably 80/20 to 99/1. If the proportion of the polymerizable monomer for shell is too low, the effect of improving the shelf stability becomes little. If the proportion is too high on the other hand, the effects of lowering the fixing temperature and improving the permeability through OHP become little.

The polymerized toner according to the present invention is composed of fine spherical particles sharp in particle diameter distribution in which the volume average particle diameter is generally 2 to 20 µm, preferably 3 to 15 µm, and the particle diameter distribution (volume average particle diameter/number average particle diameter) is generally at most 1.6, preferably at most 1.5.

The polymerized toner according to the present invention is composed of polymer particles of core-shell structure, comprising the core particles and the shell which covers each of the core particles. In the polymerized toner according to the present invention, the average thickness of the shell is generally 0.001 to 1 µm, preferably 0.005 to 0.5 µm. If the thickness of the shell is too great, the fixing ability of the toner is deteriorated. If the thickness is too small on the other hand, the shelf stability of the toner is deteriorated. The particle diameters of the core particles and the thickness of the shell in the polymerized toner can be determined by directly measuring the size and shell thickness of each of particles selected at random from electron photomicrographs thereof when they can be observed through an electron microscope. If the particle diameters of the core particles and the thickness of the shell are difficult to observe through the electron microscope, the particle diameters of the core particles are measured through the electron microscope in the same manner as described above or by means of a Coulter counter at the stage of formation of the core particles. After the core particles are then covered with the shell, the particle diameters of the resultant polymerized toner particles are measured again through the electron microscope or by means of the Coulter counter, whereby the average thickness of the shell can be found from changes in particle diameter before and after the covering with the shell. When it is difficult to measure the shell thickness by these methods, the thickness of the shell can be calculated out from the particle diameter of the core particles and the used amount of the polymerizable monomer for forming the shell.

The polymerized toner according to the present invention contains toluene-insoluble matter in an amount of generally at most 50 wt.%, preferably at most 20 wt.%, more preferably at most 10 wt.%. If the toluene-insoluble matter is contained in plenty, the fixing ability of the polymerized toner shows a tendency to lower. The toluene-insoluble matter is determined by placing a polymer component making up the polymerized toner in a 80-mesh woven metal basket, immersing the basket in toluene for 24 hours at room temperature, drying solids remaining in the basket by a vacuum drier and then measuring the weight of the dry solids to express it in terms of % by weight based on the weight of the polymer component.

The polymerized toner according to the present invention has a ratio (rl/rs) of the length (rl) to the breadth (rs) within a range of 1 to 1.2, preferably 1 to 1.15. If the ratio is too high, the resolution of an image formed from such a polymerized toner is deteriorated. In addition, when such a polymerized toner is contained in a toner container in an image forming apparatus, its durability shows a tendency to lower, since friction between particles of the polymerized toner becomes greater, and so external additives such as a flowability improver are separated from the toner.

The polymerized toner according to the present invention can be used as a developer as it is. However, it may also be used as a developer with various kinds of additives (external additives) such as a flowability improver added thereto as needed. The additives generally attach to the surface of the polymerized toner. As examples of the external additives, may be mentioned various kinds of inorganic particles and organic resin particles. Of these, silica particles and titanium oxide particles are preferred, with silica particles subjected to a hydrophobicity-imparting treatment being particularly preferred. In order to attach the external additives to the polymerized toner, in general, the external additives and the polymerized toner are charged into a mixer such as a Henschel mixer to mix them under stirring.

When the polymerized toner according to the present invention is used, the fixing temperature can be lowered to a low temperature of 80 to 150°C, preferably 80 to 130°C. In addition, the polymerized toner does not aggregate during its storage and is hence excellent in shelf stability.

### Image forming apparatus:

An image forming apparatus, to which the polymerized toner according to the present invention is applied, comprises a photosensitive member (photosensitive drum), a means for charging the surface of the photosensitive member, a means for forming an electrostatic latent image on the surface of the photosensitive member, a means for receiving a toner (developer), a means for supplying the toner to develop the electrostatic latent image on the surface of the photosensitive member, thereby forming a toner image, and a means for transferring the toner image from the surface of the photosensitive member to a transfer medium. A specific example of such an image forming apparatus is illustrated in FIG. 1.

As illustrated in FIG. 1, in the image forming apparatus, a photosensitive drum 1 as the photosensitive member is installed rotatably in the direction of an arrow A. The photosensitive drum 1 has a structure that a photoconductive layer is provided around a peripheral surface of an electroconductive support drum. The photoconductive layer is composed of, for example, an organic photosensitive member, selenium photosensitive member, zinc oxide photosensitive member or amorphous silicon photosensitive member.

Around the photosensitive drum 1, a charging roll 2 as a charging means, a laser beam irradiating device 3 as a latent image forming means, a developing roll 4 as a developing means, a transfer roll 10 as a transfer means, and optionally a cleaning device (not illustrated) are arranged along the circumferential direction of the drum.

The charging roll 2 bears an action that the surface of the photosensitive drum 1 is evenly charged either positively or negatively. Voltage is applied to the charging roll 2, and the charging roll 2 is brought into contact with the surface of the photosensitive drum 1, thereby charging the surface of the photosensitive drum 1. The charging roller 2 may be replaced by a charging means according to corona discharge.

The laser beam irradiating device 3 bears an action that light corresponding to image signals is irradiated on the surface of the photosensitive drum 1 to expose the surface of the photosensitive drum 1 evenly charged to the light on the predetermined pattern, thereby forming an electrostatic latent image on the exposed portion of the drum (in the case of reversal development) or forming an electrostatic latent image on the unexposed portion of the drum (in the case of normal development). An example of other latent image forming means includes that composed of an LED array and an optical system.

The developing roll 4 bears an action that a toner is applied to the electrostatic latent image formed on the surface of the photosensitive drum 1. Bias voltage is applied between the developing roll 4 and the photosensitive drum 1 in such a manner that the toner is applied only to a light-exposed portion of the photosensitive drum 1 in reversal development, or only to a light-unexposed portion of the photosensitive drum 1 in normal development.

In a casing 9 for receiving the toner 7, the developing roll 4 and a feed roll 6 are arranged. The developing roll 4 is arranged in close vicinity to the photosensitive drum 1 in such a manner that a part thereof comes into contact with the photosensitive drum 1, and is rotated in a direction B opposite to the rotating direction of the photosensitive drum 1. The feed roll 6 is rotated in contact with and in the same direction C as the developing roll 4 to supply the toner 7 to the outer periphery of the developing roll 4. An agitating means (agitating blade) 8 for agitating the toner is installed in the casing 9.

A blade 5 for developing roll as a layer thickness regulating means is arranged at a position between the contact point with the feed roll 6 and the contact point with the photosensitive drum 1 on the periphery of the developing roll 4. The blade 5 is composed of conductive rubber or stainless steel, and voltage of |200 V| to |600 V| is generally applied to the blade to charge the toner. Therefore, the resistivity of the blade 5 is preferably 10⁶ Ωcm or lower.

The polymerized toner 7 according to the present invention is contained in the casing 9 of the image forming apparatus. The polymerized toner 7 may comprise additives such as a flowability improver attached thereto. Since the polymerized toner according to the present invention has a core-shell structure, and the shell of the surface layer is formed of a polymer having a relatively high glass transition temperature, the stickiness of the surface is reduced, and so the polymerized toner is prevented from aggregating during storage in the casing 9. In addition, since the particle diameter distribution of the polymerized toner according to the present invention is relatively sharp, the toner layer formed on the developing roll 4 can be made a substantially single layer by the layer thickness regulating means 5, thereby forming reproducible images with good quality.

The transfer roll 10 serves to transfer the toner image formed on the surface of the photosensitive drum 1 by the developing roll 4 to a transfer medium 11. Examples of the transfer medium 1 include paper and resin sheets such as OHP sheets. As transferring means, may be mentioned a corona discharge device and a transfer belt in addition to the transfer roll 10.

The toner image transferred to the transfer medium 11 is fixed to the transfer medium by a fixing means. The fixing means is generally composed of a heating means and a press-bonding means. More specifically, the fixing means is generally composed of the combination of a heating roll (fixing roll) 12 and a press roll 13. The transfer medium 11, to which the toner image has been transferred, is passed through between the heating roll 12 and the press roll 13 to melt the toner, and at the same time press-bond it to the transfer medium 11, thereby fixing the toner image thereto.

In the image forming apparatus according to the present invention, the polymerized toner according to the present invention is used as a toner. Therefore, the toner is easily melted even when the heating temperature by the heating means is low, and is fixed to the transfer medium in a flattened state by slightly pressing it by the press-bonding means, so that high-speed printing or copying is feasible. Further, the toner image fixed to an OHP sheet is excellent in permeability through OHP.

The cleaning device serves to clean off the toner remaining on the surface of the photosensitive drum 1 without transferring and is composed of, for example, a cleaning blade or the like. The cleaning device is not always required to install in the case where a system that cleaning is conducted by the developing roll 4 at the same time as development is adopted.

### Image forming process:

In the image forming process according to the present invention, which comprises the steps of applying a toner to the surface of a photosensitive member, on which an electrostatic latent image has been formed, to make the latent image visible, and then transferring the visible image to a transfer medium, the polymerized toner according to the present invention is used as the toner.

### <EXAMPLES>

The present invention will hereinafter be described more specifically by the following Examples and Comparative Examples. However, the present invention is not limited to these examples only. Incidentally, all designations of "part" or "parts" and "%" as will be used in the following examples mean part or parts by weight and wt.% unless expressly noted.

Physical properties in the following Examples and Comparative Examples were measured in accordance with the following respective methods.

### (1) Particle diameter of toner:

The volume average particle diameter (dv) and particle diameter distribution, i.e., a ratio (dv/dp) of the volume average particle diameter to a number average particle diameter (dp) of polymer particles were measured by means of a Multisizer (manufactured by Coulter Co.). The measurement by the Multisizer was conducted under the following conditions:
aperture diameter: 50 µm;
medium: Isothone II, concentration: 15%; and
number of particles measured: 50,000 particles.

### (2) Thickness of shell:

In the examples of the present invention, the thickness of the shell in each toner sample was calculated out in the following equation though it can be measured by the Multisizer or an electron microscope where the thickness of the shell is great.

Thickness of shell (µm) = dr (1 + s/100)^{1/3} - dr wherein dr is the radius of core particles before addition of a polymerizable monomer for shell (a half of the volume average particle diameter of the core particles found from measurement by the Multisizer), and s is the number of parts of a polymerizable monomer for shell added (the number of parts per 100 parts by weight of a polymerizable monomer for core).

### (3) Volume resistivity of toner:

The volume resistivity of each toner sample was measured by means of a dielectric loss measuring device (TRS-10 Model, trade name; manufactured by Ando Electric Co., Ltd.) under conditions of a temperature of 30°C and a frequency of 1 kHz.

### (4) Fixing temperature of toner:

A commercially available printer (4 papers per minute printer) of a non-magnetic one-component development system was modified in such a manner that the temperature of a fixing roll can be varied. This modified printer was used to form an image with each toner sample, thereby evaluating the toner as to the image. A temperature at which a fixing rate of the toner amounted to 80% was defined as a fixing temperature. The fixing test was conducted by varying the temperature of the fixing roll in the printer to determine the fixing rate at each temperature, thereby finding a relationship between the temperature and the fixing rate. The fixing rate was calculated from the ratio of image densities before and after a peeling operation using a pressure-sensitive adhesive tape, which was conducted against a black solid-printed area of a test paper sheet, on which printing had been made by the modified printer. More specifically, assuming that the image density before the peeling of the adhesive tape is ID_{before}, and the image density after the peeling of the adhesive tape is ID_{after}, the fixing rate is determined by the following equation: $Fixing rate ( % ) = ( {ID}_{after} / {ID}_{before} ) x 100$

In this test, the black solid-printed area means an area controlled in such a manner that the toner is caused to adhere to all dots within this area. The peeling operation of the pressure-sensitive adhesive tape is a series of operation that a pressure-sensitive adhesive tape (Scotch Mending Tape 810-3-18, product of Sumitomo 3M Limited) is applied to a measuring area of the test paper sheet to cause the tape to adhere to the sheet by pressing the tape under a fixed pressure, and the adhesive tape is then peeled at a fixed rate in a direction along the paper sheet. The image density was measured by means of a reflection image densitometer manufactured by McBeth Co.

### (5) Shelf stability of toner:

The evaluation of shelf stability was conducted by placing each toner sample in a closed container to seal it, sinking the container into a constant-temperature water bath controlled to 50°C and then taking the container out of the water bath after a predetermined period of time went on, thereby measuring the weight of toner aggregated. The sample toner taken out of the container was transferred to a 42-mesh screen so as not to destroy the structure thereof as much as possible, and the screen was vibrated for 30 seconds by means of a powder measuring device, REOSTAT (manufactured by Hosokawa Micron Corporation) with the intensity of vibration preset to 4.5. Thereafter, the weight of the toner remaining on the screen was measured to regard it as the weight of the toner aggregated. The aggregation rate (wt.%) of the toner was calculated out from this weight of the aggregated toner and the weight of the sample.

The shelf stability of the toner sample was evaluated by 4 ranks in accordance with the following standard:
⊚: aggregation rate was lower than 5 wt.%;
O: aggregation rate was not lower than 5 wt.%, but low than 10 wt.%;
Δ: aggregation rate was not lower than 10 wt.%, but low than 50 wt.%; and
×: aggregation rate was not lower than 50 wt.%.

### (6) Permeability through OHP:

The temperature of the fixing roll in the modified printer described above was preset to 150°C to conduct printing with each toner sample on a commercially available OHP sheet (Transparency, product of Uchida Yoko Co., Ltd.), thereby evaluating the toner sample as to permeability through OHP. Whether the printed image permeated through the OHP sheet or not was visually observed, thereby ranking it as ○ where the image permeated, or × where the image did not permeate.

### (7) Charge level of toner:

The charge level of each toner sample was measured under respective environments of L/L (10°C in temperature and 20% in humidity, RH) and H/H (30°C in temperature and 80% in humidity, RH) to evaluate the toner sample as to charge level under varied environments.

The charge level of the toner was determined in the following manner. The toner was charged into a commercially available printer (4 papers per minute printer) under each of the above-described environments and left to stand for 24 hours. Thereafter, a print pattern of half tone was printed 5 times, and the toner on a developing roll was then sucked in a suction type charge level meter to measure a charge level per unit weight from the charge level and weight of the toner sucked at this time.

### (8) Evaluation of image quality:

Printing was continuously conducted with each toner sample from the beginning to count the number of printed sheets that retained an image density of 1.3 or higher as measured by a reflection densitometer (manufactured by McBeth Co) and at an unprinted area, fog of 10% or lower as measured by a whiteness meter (manufactured by Nippon Denshoku K.K.), thereby evaluating the toner sample as to image quality in accordance with the following standard:
○: the number of the printed sheets was 10,000 or more;
Δ: the number of the printed sheets was not less than 5,000, but less than 10,000; and
×: the number of the printed sheets was less than 5,000.

### [Example 1]

Stirred and mixed at 12,000 rpm in a homomixer (TK type, manufactured by Tokushu Kika Kogyo Co., Ltd.) capable of mixing with high shearing force were a polymerizable monomer (calculated Tg of the resulting copolymer = 50°C) for core composed of 78 parts of styrene and 22 parts of n-butyl acrylate, 7 parts of carbon black (Printex 150T, trade name; product of Degussa AG), 1 part of a charge control agent (Spiron Black TRH, trade name; product of Hodogaya Chemical Co., Ltd.), 0.3 parts of divinylbenzene, 0.8 parts of a polymethacrylic ester macromonomer (AA6, trade name; Tg = 94°C; product of Toagosei Chemical Industry Co., Ltd.), 10 parts of pentaerythritol tetrastearate (purity of stearic acid: about 60%) and 4 parts of t-butyl peroxy-2-ethylhexanoate, thereby uniformly dispersing them to obtain a polymerizable monomer composition (liquid mixture) for core.

On one hand, 10 parts of methyl methacrylate (calculated Tg of the resulting polymer = 105°C) and 100 parts of water were subjected to a finely dispersing treatment by an ultrasonic emulsifier, thereby obtaining an aqueous dispersion of a polymerizable monomer for shell. The droplet diameter of droplets of the polymerizable monomer for shell was found to be 1.6 µm in terms of D₉₀ as determined by means of a microtrack particle diameter distribution measuring device by adding the droplets at a concentration of 3% to a 1% aqueous solution of sodium hexametaphosphate.

On the other hand, an aqueous solution with 6.9 parts of sodium hydroxide (alkali metal hydroxide) dissolved in 50 parts of ion-exchanged water was gradually added to an aqueous solution with 9.8 parts of magnesium chloride (water-soluble polyvalent metallic salt) dissolved in 250 parts of ion-exchanged water under stirring to prepare a dispersion of colloid of magnesium hydroxide (colloid of hardly water-soluble metal hydroxide). The particle diameter distribution of the colloid formed was measured by means of the microtrack particle diameter distribution measuring device (manufactured by Nikkiso Co., Ltd.) and found to be 0.38 µm in terms of D₅₀ (50% cumulative value of number particle diameter distribution) and 0.82 µm in terms of D₉₀ (90% cumulative value of number particle diameter distribution). The measurement by means of the microtrack particle diameter distribution measuring device was performed under the following conditions:
measuring range: 0.12 to 704 µm;
measuring time: 30 seconds; and
medium: ion-exchanged water.

The polymerizable monomer composition for core prepared above was then poured into the colloidal dispersion of magnesium hydroxide obtained above, and the resultant mixture was stirred at 12,000 rpm under high shearing force by means of the TK type homomixer, thereby forming droplets of the polymerizable monomer composition for core. The thus-prepared aqueous dispersion containing droplets of the monomer composition for core was charged into a reactor equipped with an agitating blade to initiate a polymerization reaction at 90°C. At the time a conversion into a polymer reached almost 100%, the polymerizable monomer for shell prepared above and 1 part of a 1% aqueous solution of potassium persulfate were added to continue the reaction for 5 hours. Thereafter, the reaction was stopped to obtain an aqueous dispersion containing polymer particles of core-shell structure.

The volume average particle diameter (dv) of core particles measured by taking out them just before the polymerizable monomer for shell was added was 5.7 µm, and a ratio of the volume average particle diameter (dv) to the number average particle diameter (dp) thereof was 1.32. The resultant polymer particles had a shell thickness of 0.09 µm and an rl/rs ratio of 1.1 and contained 2% of toluene-insoluble matter.

While stirring the above-obtained aqueous dispersion of the polymer particles of core-shell structure, the pH of the system was adjusted to 4 or lower with sulfuric acid to conduct acid washing (25°C, 10 minutes). After water was separated by filtration from the dispersion, 500 parts of ion-exchanged water were newly added to form a slurry again, and the slurry was washed with water. Thereafter, the dehydration and water washing were repeated several times, and solids were then collected by filtration. The thus-collected solids were dried at 45°C for 24 hours by a dryer to obtain polymer particles (polymerized toner).

To 100 parts of the polymerized toner of core-shell structure obtained above were added 0.3 parts of colloidal silica (R-972, trade name; product of Nippon Aerosil Co., Ltd.) subjected to a hydrophobicity-imparting treatment, and they were mixed by means of a Henschel mixer to prepare a non-magnetic one-component developer (hereinafter referred to as a developer or toner merely). The volume resistivity of the toner thus obtained was measured and found to be 11.3 logΩ·cm.

The toner thus obtained was used to measure its fixing temperature. As a result, it was 120°C. The shelf stability of the toner was extremely good (rank = ⊚). The evaluation of image revealed that an image high in image density, free of fog and irregularities, and extremely good in resolution was obtained. The results are shown in Table 1.

### [Example 2]

A polymerized toner and a developer (toner) were obtained in the same manner as in Example 1 except that the amount of pentaerythritol tetrastearate used in Example 1 was changed to 5 parts. The evaluation of image revealed that an image high in image density, free of fog and irregularities, and extremely good in resolution was obtained. The results are shown in Table 1.

### [Example 3]

A polymerized toner and a developer (toner) were obtained in the same manner as in Example 1 except that pentaerythritol tetrastearate used in Example 1 was changed to glycerol triarachidate (purity of arachidic acid: about 60%). The results are shown in Table 1.

### [Comparative Example 1]

A polymerized toner and a developer (toner) were obtained in the same manner as in Example 1 except that pentaerythritol tetrastearate used in Example 1 was changed to paraffin wax having a melting point of 60°C. The results are shown in Table 1.

### [Comparative Example 2]

A polymerized toner and a developer (toner) were obtained in the same manner as in Example 1 except that pentaerythritol tetrastearate used in Example 1 was changed to low molecular weight polypropylene having a number average molecular weight of 2,200. The results are shown in Table 1.

**Table 1**

| | Example | | | Comp. Ex. | |
|---|---|---|---|---|---|
| | 1 | 2 | 3 | 1 | 2 |
| Core particles: | | | | | |
| dv [µm] | 5.7 | 5.7 | 6.1 | 6.5 | 6.0 |
| dv/dp | 1.32 | 1.28 | 1.25 | 1.35 | 1.22 |
| Polymer particles: | | | | | |
| Thickness of shell [µm] | 0.09 | 0.09 | 0.09 | 0.10 | 0.10 |
| Toluene-insoluble matter [%] | 2 | 3 | 3 | 2 | 4 |
| Evaluation of toner: | | | | | |
| dv [µm] | 5.9 | 5.9 | 6.3 | 6.7 | 6.2 |
| dv/dp | 1.30 | 1.30 | 1.28 | 1.36 | 1.24 |
| Volume resistivity [logΩcm] | 11.3 | 11.4 | 11.2 | 11.0 | 11.4 |
| Fixing temperature [°C] | 120 | 130 | 130 | 150 | 160 |
| Shelf stability | ⊚ | ⊚ | ⊚ | Δ | Δ |
| Charge level under L/L [µc/g] | -26 | -24 | -28 | -25 | -27 |
| Charge level under H/H [µc/g] | -16 | -25 | -25 | -20 | -25 |
| Evaluation of image quality | ○ | ○ | ○ | × | Δ |

### [Comparative Example 3]

Four parts of saturated polyester, 83 parts of styrene, 17 parts of butyl acrylate, 7 parts of carbon black, 1 part of a metal compound of salicylic acid and 10 parts of pentaerythritol dibehenate diacetate were dispersed by means of the TK type homomixer, and 5 parts of 2,2'-azobis(2,4-dimethylvaleronitrile) were added to the resultant dispersion, thereby preparing a polymerizable monomer composition. After the polymerizable monomer composition was then granulated, it was heated to 60°C to conduct polymerization for 10 hours. After the polymerization, the formed product was washed and dried to obtain polymer particles (polymerized toner). A developer (toner) was obtain in the same manner as in Example 1 except that this polymerized toner was used. The results are shown in Table 2.

### [Example 4]

A polymerized toner and a developer (toner) were obtained in the same manner as in Example 1 except that 10 parts of methyl methacrylate used as the polymerizable monomer for shell in Example 1 were changed to 9 parts of methyl methacrylate and 1 part of butyl acrylate. The evaluation results are shown in Table 2.

### [Example 5]

A polymerized toner and a developer (toner) were obtained in the same manner as in Example 1 except that 10 parts of styrene were used in place of 10 parts of methyl methacrylate used as the polymerizable monomer for shell in Example 1, and 20 parts of methanol were added just before the polymerizable monomer for shell was added. The evaluation results are shown in Table 2.

### [Example 6]

A polymerized toner and a developer (toner) were obtained in the same manner as in Example 1 except that 2,2-azobisisobutyronitrile was used in place of t-butyl peroxy-2-ethylhexanoate used as the polymerization initiator for the polymerizable monomer for core in Example 1, and the reaction temperature was changed to 75°C. The results are shown in Table 2. When this developer was used to conduct fixing, slight odor was given off.

### [Example 7]

A polymerized toner and a developer (toner) were obtained in the same manner as in Example 1 except that the polymerizable monomer for shell was added without conducting the treatment by means of the ultrasonic emulsifier in Example 1. The results are shown in Table 2.

**Table 2**

| | Example | | | | Comp. Ex. |
|---|---|---|---|---|---|
| | 4 | 5 | 6 | 7 | 3 |
| Core particles: | | | | | |
| dv [µm] | 6.0 | 6.1 | 5.9 | 6.5 | 6.2 |
| dv/dp | 1.27 | 1.31 | 1.35 | 1.40 | 1.38 |
| Polymer particles: | | | | | |
| Thickness of shell [µm] | 0.10 | 0.10 | 0.09 | 0.10 | 0.09 |
| Toluene-insoluble matter [%] | 3 | 3 | 5 | 4 | 4 |
| Evaluation of toner: | | | | | |
| dv [µm] | 6.2 | 6.3 | 6.1 | 6.7 | 6.4 |
| dv/dp | 1.27 | 1.31 | 1.33 | 1.40 | 1.37 |
| Volume resistivity [logΩcm] | 11.3 | 11.4 | 11.2 | 11.1 | 11.1 |
| Fixing temperature [°C] | 120 | 130 | 130 | 130 | 140 |
| Shelf stability | ⊚ | ⊚ | ⊚ | ○ | × |
| Charge level under L/L [µc/g] | -27 | -30 | -22 | -23 | -20 |
| Charge level under H/H [µc/g] | -22 | -27 | -18 | -19 | -17 |
| Evaluation of image quality | ○ | ○ | ○ | ○ | × |

### [Example 8]

A polymerized toner and a developer (toner) were obtained in the same manner as in Example 1 except that butyl acrylate used as the polymerizable monomer for core in Example 1 was changed to 2-ethylhexyl acrylate. The results are shown in Table 3.

### [Example 9]

A polymerized toner and a developer (toner) were obtained in the same manner as in Example 1 except that 5 parts of a magenta pigment (Pigment Red 122) were used in place of 7 parts of carbon black used in Example 1. The results are shown in Table 3.

### [Example 10]

A polymerized toner and a developer (toner) were obtained in the same manner as in Example 1 except that 5 parts of a yellow quinophthalone pigment (Pigment Yellow 138) were used in place of 7 parts of carbon black used in Example 1. The results are shown in Table 3.

### [Example 11]

A polymerized toner and a developer (toner) were obtained in the same manner as in Example 1 except that 5 parts of a cyan pigment (Pigment Blue 15:3) were used in place of 7 parts of carbon black used in Example 1. The results are shown in Table 3.

### [Comparative Example 4]

A polymerized toner and a developer (toner) were obtained in the same manner as in Comparative Example 1 except that 5 parts of a magenta pigment (Pigment Red 122) were used in place of 7 parts of carbon black used in Example 1. The results are shown in Table 3.

**Table 3**

| | Example | | | | Comp. Ex. |
|---|---|---|---|---|---|
| | 8 | 9 | 10 | 11 | 4 |
| Core particles: | | | | | |
| dv [µm] | 6.3 | 6.1 | 6.2 | 6.5 | 5.9 |
| dv/dp | 1.21 | 1.18 | 1.25 | 1.31 | 1.27 |
| Polymer particles: | | | | | |
| Thickness of shell [µm] | 0.10 | 0.10 | 0.10 | 0.10 | 0.09 |
| Toluene-insoluble matter [%] | 3 | 4 | 5 | 6 | 4 |
| Evaluation of toner: | | | | | |
| dv [µm] | 6.5 | 6.3 | 6.4 | 6.7 | 6.1 |
| dv/dp | 1.22 | 1.17 | 1.24 | 1.29 | 1.27 |
| Volume resistivity [logΩcm] | 11.4 | 12.5 | 12.4 | 11.6 | 12.4 |
| Fixing temperature [°C] | 120 | 130 | 120 | 130 | 130 |
| Shelf stability | ⊚ | ⊚ | ⊚ | ⊚ | Δ |
| Charge level under L/L [µc/g] | -28 | -32 | -34 | -28 | -33 |
| Charge level under H/H [µc/g] | -25 | -30 | -31 | -25 | -29 |
| Permeability through OHP | - | ○ | ○ | ○ | ○ |
| Evaluation of image quality | ○ | ○ | ○ | ○ | × |

### [Example 12]

A polymerized toner and a developer (toner) were obtained in the same manner as in Example 1 except that pentaerythritol tetramyristate was used in place of pentaerythritol tetrastearate used in Example.

The volume average particle diameter (dv) of core particles measured by taking out them just before the polymerizable monomer for shell was added was 5.8 µm, and a ratio of the volume average particle diameter (dv) to the number average particle diameter (dp) thereof was 1.22. The resultant polymer particles had a shell thickness of 0.09 µm and an rl/rs ratio of 1.1 and contained 2% of toluene-insoluble matter.

The volume resistivity of the non-magnetic one-component developer (toner) obtained by adding colloidal silica subjected to the hydrophobicity-imparting treatment to the polymerized toner was 11.3 logΩ·cm. The toner was used to measure its fixing temperature. As a result, it was 120°C. The shelf stability of the toner was extremely good (rank = ⊚). The toner had charge levels of -28 µc/g and -25 µc/g under L/L and H/H environments, respectively. The evaluation of image revealed that an image high in image density, free of fog and irregularities, and extremely good in resolution was obtained (rank of image quality = ○).

Incidentally, pentaerythritol tetramyristate was excellent in solubility in the polymerizable monomer compared with pentaerythritol tetrastearate, and so there was no need to grind or melt it in advance for enhancing the solubility at room temperature.

### <INDUSTRIAL APPLICABILITY>

According to the present invention, there are provided polymerized toners which have a low fixing temperature and uniformly melting ability, and moreover are excellent in shelf stability, and a production process thereof. The use of the polymerized toners according to the present invention permits the speeding-up of copying or printing, the formation of full-color images and energy saving. The polymerized toners according to the present invention can form toner images which exhibit excellent permeability when conducting printing on an OHP sheet with such a polymerized toner and fixing the resulting image thereto. The polymerized toners according to the present invention permit the formation of high-quality images without causing fogging and deterioration of image density. According to the present invention, there are provided an image forming process comprising using the polymerized toner(s) having such excellent various properties, and an image forming apparatus in which the polymerized toner(s) are received.

## Claims

1. A polymerized toner of core-shell structure, comprising core particles composed of colored polymer particles, which comprise a polyfunctional ester compound, a colorant and a polymer component, and, having each of the core particles, a shell which is formed of a polymer having a glass transition temperature higher than that of the polymer component making up the core particles,
wherein the polyfunctional ester compound is an ester formed of a trifunctional or still higher polyfunctional polyhydric alcohol and a carboxylic acid having 10 to 30 carbon atoms, and
wherein the polymer component making up the core particles has a glass transition temperature of 80°C or lower, the shell is a polymer layer formed on the core particle surface by subjecting a polymerizable monomer for shell, which is capable of forming polymer having a glass transition temperature higher than 80°C, to suspension polymerization in the presence of the core particles to form a glass shell polymer having a glass transition temperature in the range 80 to 110°C, and a difference in glass transition temperature between the polymer component making up the core particles and the polymer making up the shell is at least 10°C.

2. The polymerized toner according to claim 1, wherein the core particles are colored polymer particles obtained by subjecting a polymerizable monomer composition containing a polymerizable monomer for core, the polyfunctional ester compound formed of the polyhydric alcohol and the carboxylic acid, and the colorant to suspension polymerization, preferably in the presence of a macromonomer.

3. The polymerized toner according to claim 1 or 2, wherein the core particle have an average particle diameter of 0.5 to 20 µm, and the shell has an average thickness of 0.001 to 1 µm.

4. The polymerized toner according to any preceding claim, which has a volume average particle diameter of 2 to 20 µm and a particle diameter distribution (volume average particle diameter/number average particle diameter) of at most 1.6.

5. The polymerized toner according to any preceding claim, wherein the polyfunctional ester compound is contained in a proportion of 0.1 to 40 parts by weight per 100 parts by weight of the polymer component making up the core particles.

6. The polymerized toner according to any preceding claim, wherein the polyfunctional ester compound is a compound represented by the formula (I): wherein R¹, R², R³ and R⁴ are independently an alkyl group or phenyl group, and the number of carbon atoms of the alkyl group or phenyl group is 10 to 30, and is preferably pentaerythritol tetrastearate or pentaerythritol tetramyristate.

7. A process for producing a polymerized toner of core-shell structure, which comprises the steps of (1) subjecting a polymerizable monomer composition containing a polyfunctional ester compound formed of a trifunctional or still higher polyfunctional polyhydric alcohol and a carboxylic acid having 10 to 30 carbon atoms, a colorant , and a polymerizable monomer for core, which is capable of forming a polymer component having a glass transition temperature of 80°C or lower, to suspension polymerization using an oil-soluble radical polymerization initiator in an aqueous dispersion medium containing a dispersing agent to prepare core particles formed of colored polymer particles; and then (2) subjecting polymerization monomer for shell, which is capable of forming a polymer having a glass transition temperature higher than 80°C, to suspension polymerization using a water-soluble radical polymerization initiator in the presence of the core particles, thereby forming a shell which is formed of a polymer having a glass transition temperature higher than that of a polymer component making up the core particles and covers each of the core particles, wherein a difference in glass transition temperature between the polymer component formed from the polymerizable monomer for core and the polymer formed from the polymerizable monomer for shell is at least 10°C and the glass transition temperature of the shell polymer is in the range 80 to 110°C.

8. The production process according to claim 7, wherein in the step (1), the polymerizable monomer composition is subjected to the suspension polymerization in the presence of a macromonomer to prepare core particles formed of colored polymer particles, and preferably the macromonomer has a number average molecular weight of 1,000 to 30,000 and a glass transition temperature higher than that of the polymer obtained by polymerizing the polymerizable monomer for core.

9. The production process according to claim 8, wherein the macromonomer is used in an amount of 0.01 to 10 parts by weight per 100 parts by weight of the polymerizable monomer for core.

10. The production process according to claims 7 to 9, wherein the polyfunctional ester compound is contained in a proportion of 0.1 to 40 parts by weight per 100 pans by weight of the polymerizable monomer for core.

11. The production process according to any of claims 7 to 10, wherein the polyfunctional ester compound is a compound represented by the formula (I): wherein R¹, R², R³ and R⁴ are independently an alkyl group or phenyl group, and the number of carbon atoms of the alkyl group or phenyl group is 10 to 30, and is preferably pentaerythritol tetrastearate or pentaerythritol tetramyrisiate.

12. The production process according to any of claims 7 to 11, wherein the polymerizable monomer composition further comprises a crosslinking monomer.

13. The production process according to any of claims 7 to 12, wherein the oil-soluble radical polymerization initiator is an organic peroxide whose ten-hour half-life temperature is 60 to 80°C, and whose molecular weight is 250 or lower.

14. The production process according to any of claims 7 to 13, wherein in the step (1), the suspension polymerization is conducted in an aqueous dispersion medium containing a colloid of a hardly water-soluble metal hydroxide as the dispersing agent.

15. The production process according to claim 14, wherein the colloid of the hardly water-soluble metal hydroxide is such that the 50% cumulative value (D₅₀) of the number particle diameter distribution thereof is at most 0.5 µm, and the 90% cumulative value (D₉₀) of number particle diameter distribution thereof is at most 1 µm.

16. The production process according to claim 14, wherein the colloid of the hardly water-soluble metal hydroxide is obtained by adjusting the pH of an aqueous solution of a water-soluble polyvalent metallic compound to 7 or higher.

17. The production process according to claim 15, wherein the colloid of the hardly water-soluble metal hydroxide is obtained by reacting a water-soluble polyvalent metallic compound with an alkali metal hydroxide in an aqueous phase.

18. The production process according to Claim 7, wherein in the step (1), a liquid mixture containing at least the polyfunctional ester compound, the colorant, the polymerizable monomer for core and a radical polymerization initiator is prepared, the liquid mixture is poured into the aqueous dispersion medium containing the dispersing agent to form minute droplets under stirring, and the suspension polymerization is then conducted at a temperature of 30 to 200°C.

19. The production process according to any of clams 7 to 18, wherein in the step (1), core particles composed of colored polymer particles having a volume average particle diameter (dv) of 0.5 to 20 µm and a ratio (dv/dp) of the volume average particle diameter (dv) to a number average particle diameter (dp) of at most 1.7 are prepared.

20. The production process according to any of claims 7 to 19, wherein in the step (2), the polymerizable monomer for shell is prepared into droplets having a number average droplet diameter smaller than the core particles and then subjected to the suspension polymerization.

21. The production process according to any of claims 7 to 20, wherein the polymerizable monomer for shell is a monomer having a solubility of at least 0.1 wt.% in water at 20°C.

22. The production process according to any of claims 7 to 20, wherein the polymerizable monomer for shell is a monomer having a solubility lower than 0.1 wt. % in water at 20°C, and in the step (2), said polymerizable monomer for shell and an organic solvent having a solubility of at least 5 wt.% in water at 20°C are added to conduct the suspension polymerization.

23. The production process according to any of claims 7 to 22, wherein in the step (2), the polymerizable monomer for shell and a charge control agent are added to conduct the suspension polymerization.

24. The production process according to any of claims 7 to 23, wherein in the step (2), shell formed of a polymer layer having an average film thickness of 0.001 to 1 µm is formed.

25. An image forming process, comprising the steps of applying a toner to the surface of a photosensitive member, on which an electrostatic latent image has been formed, to make the latent image visible, and then transferring the visible image to a transfer medium, wherein the toner is a polymerized toner as defined in any of claims 1 to 6.

26. Use of a polymerized toner as defined in any claims 1 to 6 in an image forming apparatus comprising a photosensitive member, a means for charging the surface of the photosensitive member, a means for forming an electrostatic latent image on the surface of the photosensitive member, a means for receiving a toner, a means for supplying the toner to develop the electrostatic latent image on the surface of the photosensitive member, thereby forming a toner image, and a means for transferring the toner image from the surface of the photosensitive member to a transfer medium.

## Patentansprüche

1. Polymerisierter Toner mit einem Kem-Hülle-Aufbau, der Kernteilchen umfasst, die aus farbigen Polymerteilchen zusammengesetzt sind, die eine polyfunktionelle Esterverbindung, einen Farbstoff und einen Polymerbestandteil umfassen, und, jedes der Kernteilchen aufweisend, eine Hülle, die aus einem Polymer besteht, dessen Glasübergangstemperatur höher ist als die des Polymerbestandteils, aus dem die Kernteilchen bestehen,
wobei die polyfunktionelle Esterverbindung ein Ester ist, der aus einem trifunktionellen oder noch höheren polyfunktionellen mehrwertigen Alkohol und einer Carbonsäure besteht, die 10 bis 30 Kohlenstoffatome aufweist, und
wobei der Polymerbestandteil, aus dem die Kernteilchen bestehen, eine Glasübergangstemperatur von 80 °C oder weniger aufweist, die Hülle eine Polymerschicht ist, die auf der Kernteilchenoberfläche gebildet wird, indem ein polymerisierbares Monomer für die Hülle, das ein Polymer mit einer höheren Glasübergangstemperatur als 80 °C bilden kann, in Gegenwart der Kernteilchen einer Suspensionspolymerisation unterworfen wird, um ein Glashüllenpolymer zu bilden, das eine Glasübergangstemperatur im Bereich 80 bis 110 °C aufweist, und ein Unterschied der Glasübergangstemperatur zwischen dem Polymerbestandteil, aus dem die Kernteilchen bestehen, und dem Polymer, aus dem die Hülle besteht, mindestens 10 °C beträgt.

2. Polymerisierter Toner nach Anspruch 1, wobei die Kernteilchen farbige Polymerteilchen sind, die erhalten werden, indem eine polymerisierbare Monomerzusammensetzung, die ein polymerisierbares Monomer für die Hülle, die polyfunktionelle Esterverbindung, die aus dem mehrwertigen Alkohol und der Carbonsäure besteht, und den Farbstoff enthält, vorzugsweise in Gegenwart eines Makromonomers einer Suspensionspolymerisation unterworfen wird.

3. Polymerisierter Toner nach Anspruch 1 oder 2, wobei die Kernteilchen einen durchschnittlichen Teilchendurchmesser von 0,5 bis 20 µm aufweisen und die Hülle eine durchschnittliche Dicke von 0,001 bis 1 µm aufweist.

4. Polymerisierter Toner nach einem der vorhergehenden Ansprüche, der einen Volumenmittelwert des Teilchendurchmessers von 2 bis 20 µm und eine Verteilung des Teilchendurchmessers (Volumenmittelwert des Teilchendurchmessers /Zahlenmittelwert des Teilchendurchmessers) von höchstens 1,6 aufweist.

5. Polymerisierter Toner nach einem der vorhergehenden Ansprüche, wobei die polyfunktionelle Esterverbindung in einem Anteil von 0,1 bis 40 Gewichtsteilen auf 100 Gewichtsteile des Polymerbestandteils, aus dem die Kernteilchen bestehen, enthalten ist.

6. Polymerisierter Toner nach einem der vorhergehenden Ansprüche, wobei die polyfunktionelle Esterverbindung eine Verbindung ist, die mit der Formel (I) wiedergegeben wird: wobei R¹, R², R³ und R⁴ unabhängig eine Alkylgruppe oder Phenylgruppe sind und die Anzahl von Kohlenstoffatomen der Alkylgruppe oder Phenylgruppe 10 bis 30 beträgt, und vorzugsweise Pentaerythrit-Tetrastearat oder Pentaerythrit-Tetramyristat ist.

7. Verfahren zum Herstellen eines polymerisierten Toners mit einem Kern-Hülle-Aufbau, das die folgenden Schritte umfasst: (1) Suspensionspolymerisation einer polymerisierbaren Monomerzusammensetzung, die eine polyfunktionelle Esterverbindung, die aus einem trifunktionellen oder noch höheren polyfunktionellen mehrwertigen Alkohol und einer Carbonsäure besteht, die 10 bis 30 Kohlenstoffatome aufweist, einen Farbstoff und ein polymerisierbares Monomer für den Kern enthält, das einen Polymerbestandteil mit einer Glasübergangstemperatur von 80 °C oder niedriger bilden kann, unter Verwendung eines öllöslichen radikalischen Polymerisationsinitiators in einem wässrigen Dispersionsmedium, das ein Dispersionsmittel enthält, um Kernteilchen herzustellen, die aus farbigen Polymerteilchen bestehen; und anschließend (2) Suspensionspolymerisation des Polymerisationsmonomers für die Hülle, das ein Polymer mit einer höheren Glasübergangstemperatur als 80 °C bilden kann, unter Verwendung eines wasserlöslichen radikalischen Polymerisationsinitiators in Gegenwart der Kernteilchen, wodurch eine Hülle entsteht, die aus einem Polymer besteht, dessen Glasübergangstemperatur höher als die eines Polymerbestandteils ist, aus dem die Kernteilchen bestehen, und jedes der Kernteilchen bedeckt, wobei ein Unterschied der Glasübergangstemperatur zwischen dem Polymerbestandteil, der aus dem polymerisierbaren Monomer für den Kern besteht, und dem Polymer, das aus dem polymerisierbaren Monomer für die Hülle besteht, mindestens 10 °C beträgt und die Glasübergangstemperatur des Hüllenpolymers im Bereich von 80 bis 110 °C liegt.

8. Herstellungsverfahren nach Anspruch 7, wobei in Schritt (1) die polymerisierbare Monomerzusammensetzung in Gegenwart eines Makromonomers der Suspensionspolymerisation unterworfen wird, um Kernteilchen herzustellen, die aus farbigen Polymerteilchen bestehen, und das Makromonomer vorzugsweise einen Zahlenmittelwert der Molekülmasse von 1.000 bis 30.000 und eine Glasübergangstemperatur aufweist, die höher ist als die des Polymers, das durch Polymerisation des polymerisierbaren Monomers für den Kern erhalten wird.

9. Herstellungsverfahren nach Anspruch 8, wobei das Makromonomer in einer Menge von 0,01 bis 10 Gewichtsteilen auf 100 Gewichtsteile des polymerisierbaren Monomers für den Kern verwendet wird.

10. Herstellungsverfahren nach den Ansprüchen 7 bis 9, wobei die polyfunktionelle Esterverbindung in einem Anteil von 0,1 bis 40 Gewichtsteilen auf 100 Gewichtsteile des polymerisierbaren Monomers für den Kern enthalten ist.

11. Herstellungsverfahren nach einem der Ansprüche 7 bis 10, wobei die polyfunktionelle Esterverbindung eine Verbindung ist, die mit der Formel (I) wiedergegeben wird: wobei R¹, R², R³ und R⁴ unabhängig eine Alkylgruppe oder Phenylgruppe sind und die Anzahl von Kohlenstoffatomen der Alkylgruppe oder Phenylgruppe 10 bis 30 beträgt, und vorzugsweise Pentaerythrit-Tetrastearat oder Pentaerythrit-Tetramyristat ist.

12. Herstellungsverfahren nach einem der Ansprüche 7 bis 11, wobei die polymerisierbare Monomerzusammensetzung ferner ein Vernetzungsmonomer umfasst.

13. Herstellungsverfahren nach einem der Ansprüche 7 bis 12, wobei der öllösliche radikalische Polymerisationsinitiator ein organisches Peroxid ist, dessen Temperatur, bei der die Halbwertszeit zehn Stunden beträgt, 60 bis 80 °C beträgt und dessen molekulare Masse 250 oder geringer ist.

14. Herstellungsverfahren nach einem der Ansprüche 7 bis 13, wobei in Schritt (1) die Suspensionspolymerisation in einem wässrigen Dispersionsmedium durchgeführt wird, das ein Kolloid aus einem in Wasser kaum löslichen Metallhydroxid als Dispersionsmittel enthält.

15. Herstellungsverfahren nach Anspruch 14, wobei das Kolloid aus dem in Wasser kaum löslichen Metallhydroxid derart ist, dass sein 50%-Summenwert (D₅₀) der Anzahlverteilung des Teilchendurchmessers höchstens 0,5 µm beträgt und sein 90%-Summenwert (D₉₀) der Anzahlverteilung des Teilchendurchmessers höchstens 1 µm beträgt.

16. Herstellungsverfahren nach Anspruch 14, wobei das Kolloid aus dem in Wasser kaum löslichen Metallhydroxid durch Einstellen des pH einer wässrigen Lösung einer wasserlöslichen mehrwertigen Metallverbindung auf 7 oder mehr erhalten wird.

17. Herstellungsverfahren nach Anspruch 15, wobei das Kolloid aus dem in Wasser kaum löslichen Metallhydroxid durch zur Reaktion Bringen einer wasserlöslichen mehrwertigen Metallverbindung mit einem Alkalimetallhydroxid in einer wässrigen Phase erhalten wird.

18. Herstellungsverfahren nach Anspruch 7, wobei in Schritt (1) ein Flüssigkeitsgemisch, das mindestens die polyfunktionelle Esterverbindung, den Farbstoff, das polymerisierbare Monomer für den Kern und einen radikalischen Polymerisationsinitiator enthält, hergestellt wird, das Flüssigkeitsgemisch in das wässrige Dispersionsmedium, das das Dispersionsmittel enthält, gegossen wird, um unter Rühren winzige Tröpfchen zu bilden, und die Suspensionspolymerisation anschließend bei einer Temperatur von 30 bis 200 °C durchgeführt wird.

19. Herstellungsverfahren nach einem der Ansprüche 7 bis 18, wobei in Schritt (1) Kernteilchen, die aus farbigen Polymerteilchen mit einem Volumenmittelwert des Teilchendurchmessers (dv) von 0,5 bis 20 µm und einem Verhältnis (dv/dp) des Volumenmittelwerts des Teilchendurchmessers (dv) zum Zahlenmittelwert des Teilchendurchmessers (dp) von höchstens 1,7 zusammengesetzt sind, hergestellt werden.

20. Herstellungsverfahren nach einem der Ansprüche 7 bis 19, wobei in Schritt (2) das polymerisierbare Monomer für die Hülle als Tröpfchen mit einem Zahlenmittelwert des Tröpfchendurchmessers, der geringer ist als die Kernteilchen, hergestellt und anschließend der Suspensionspolymerisation unterworfen wird.

21. Herstellungsverfahren nach einem der Ansprüche 7 bis 20, wobei das polymerisierbare Monomer für die Hülle ein Monomer mit einer Löslichkeit in Wasser bei 20 °C von mindestens 0,1 Gew.-% ist.

22. Herstellungsverfahren nach einem der Ansprüche 7 bis 20, wobei das polymerisierbare Monomer für die Hülle ein Monomer mit einer Löslichkeit in Wasser bei 20 °C von unter 0,1 Gew.-% ist und dieses polymerisierbare Monomer für die Hülle und ein organisches Lösungsmittel mit einer Löslichkeit in Wasser bei 20 °C von mindestens 5 Gew.-% in Schritt (2) zugegeben werden, um die Suspensionspolymerisation durchzuführen.

23. Herstellungsverfahren nach einem der Ansprüche 7 bis 22, wobei das polymerisierbare Monomer für die Hülle und ein Ladungssteuermittel in Schritt (2) zugegeben werden, um die Suspensionspolymerisation durchzuführen.

24. Herstellungsverfahren nach einem der Ansprüche 7 bis 23, wobei in Schritt (2) die Hülle, die aus einer Polymerschicht mit einer durchschnittlichen Schichtdicke von 0,001 bis 1 µm besteht, erzeugt wird.

25. Bilderzeugungsverfahren, das die Schritte des Aufbringens eines Toners auf die Oberfläche eines lichtempfindlichen Elements, auf dem ein elektrostatisches latentes Bild erzeugt wurde, umfasst, um das latente Bild sichtbar zu machen, und anschließend das Übertragen des sichtbaren Bilds auf ein Übertragungsmedium, wobei der Toner ein polymerisierter Toner nach einem der Ansprüche 1 bis 6 ist.

26. Verwendung eines polymerisierten Toners nach einem der Ansprüche 1 bis 6 in einer bilderzeugenden Vorrichtung, die ein lichtempfindliches Element, ein Mittel zum Aufladen der Oberfläche des lichtempfindlichen Elements, ein Mittel zum Erzeugen eines elektrostatischen latenten Bilds auf der Oberfläche des lichtempfindlichen Elements, ein Mittel zum Aufnehmen eines Toners, ein Mittel zum Bereitstellen des Toners zum Entwickeln des elektrostatischen latenten Bilds auf der Oberfläche des lichtempfindlichen Elements, wodurch ein Tonerbild entsteht, und ein Mittel zum Übertragen des Tonerbilds von der Oberfläche des lichtempfindlichen Elements auf ein Übertragungsmedium umfasst.

## Revendications

1. Toner polymérisé de structure coeur-coque, comprenant des particules de coeur composées de particules polymères colorées, qui comprennent un composé ester polyfonctionnel, un colorant et un composant polymère, et chacune des particules de coeur ayant une coque, qui est formée d'un polymère ayant une température de transition vitreuse supérieure à celle du composant polymère constituant les particules de coeur,
où le composé ester polyfonctionnel est un ester formé d'un alcool polyhydroxylé trifonctionnel ou de plus haute fonctionnalité et d'un acide carboxylique ayant 10 à 30 atomes de carbone, et
où le composant polymère constituant les particules de coeur a une température de transition vitreuse de 80°C
ou moins, la coque est une couche polymère formée sur la surface de la particule de coeur en soumettant un monomère polymérisable de la coque, qui est capable de former un polymère ayant une température de transition vitreuse supérieure à 80°C, à une polymérisation en suspension en présence des particules de coeur, pour former une coque vitreuse de polymère ayant une température de transition vitreuse située dans l'intervalle allant de 80°C à 110°C, et où la différence de température de transition vitreuse entre le composant polymère constituant les particules de coeur et le polymère constituant la coque est d'au moins 10°C.

2. Toner polymérisé selon la revendication 1, où les particules de coeur sont des particules polymères colorées, obtenues en soumettant une composition de monomère polymérisable, contenant un monomère polymérisable pour le coeur, le composé ester polyfonctionnel formé de l'alcool polyhydroxylé et de l'acide carboxylique, et du colorant, à une polymérisation en suspension, de préférence en présence d'un macromonomère.

3. Toner polymérisé selon la revendication 1 ou 2, où les particules de coeur ont un diamètre particulaire moyen allant de 0,5 à 20 µm, et la coque a une épaisseur moyenne allant de 0,001 à 1 µm.

4. Toner polymérisé selon l'une quelconque des revendications précédentes, qui a un diamètre particulaire moyen en volume allant de 2 à 20 µm, et une distribution du diamètre particulaire (diamètre particulaire moyen en volume/ diamètre particulaire moyen en nombre) d'au plus 1,6.

5. Toner polymérisé selon l'une quelconque des revendications précédentes, où le composé ester polyfonctionnel est présent en une proportion allant de 0,1 à 40 parties en poids par 100 parties en poids du composant polymère constituant les particules de coeur.

6. Toner polymérisé selon l'une quelconque des revendications précédentes, où le composé ester polyfonctionnel est un composé représenté par la formule (I) : où R¹, R², R³ et R⁴ sont indépendamment un radical alkyle ou un radical phényle, et le nombre d'atomes de carbone du radical alkyle ou du radical phényle se situe dans l'intervalle allant de 10 à 30, et est de préférence le tétrastéarate de pentaérythritol ou le tétramyristate de pentaérythritol.

7. Procédé de production d'un toner polymérisé de structure coeur-coque, qui comprend les étapes qui consistant à (1) soumettre une composition de monomère polymérisable, contenant un composé ester polyfonctionnel formé d'un alcool polyhydroxylé trifonctionnel ou de fonctionnalité supérieure et d'un acide carboxylique ayant 10 à 30 atomes de carbones, d'un colorant, et d'un monomère polymérisable pour le coeur, qui est capable de former un composant polymère ayant une température de transition vitreuse de 80°C ou moins, à une polymérisation en suspension à l'aide d'un initiateur de polymérisation radicalaire oléo-soluble dans un milieu de dispersion aqueux contenant un agent dispersant, pour préparer des particules de coeur formées de particules polymères colorées, puis (2) soumettre le monomère de polymérisation pour la coque, qui est capable de former un polymère ayant une température de transition vitreuse supérieure à 80°C, à une polymérisation en suspension à l'aide d'un initiateur de polymérisation radicalaire hydrosoluble, en présence des particules de coeur, pour former une coque qui est formée d'un polymère ayant une température de transition vitreuse supérieure à celle d'un composant polymère constituant les particules de coeur, et qui couvre chacune des particules de coeur, où une différence de température de transition vitreuse entre le composant polymère formé du monomère polymérisable du coeur et le polymère formé du monomère polymérisable pour la coque est d'au moins 10°C, et la température de transition vitreuse du polymère de coque se situe dans l'intervalle allant de 80 à 110°C.

8. Procédé de production selon la revendication 7, où dans l'étape (1), la composition de monomère polymérisable est soumise à la polymérisation en suspension en présence d'un macromonomère pour préparer des particules de coeur, formées de particules polymères colorées, et de préférence, le macromère a un poids moléculaire moyen en nombre allant de 1000 à 30 000 et une température de transition vitreuse supérieure à celle du polymère obtenu par polymérisation du monomère polymérisable pour le coeur.

9. Procédé de production selon la revendication 8, où le macromonomère est utilisé en une quantité allant de 0,01 à 10 parties en poids par 100 parties en poids du monomère polymérisable pour le coeur.

10. Procédé de production selon les revendications 7 à 9, où le composé ester polyfonctionnel est présent en une proportion allant de 0,1 à 40 parties en poids par 100 parties en poids du monomère polymérisable pour le coeur.

11. Procédé de production selon l'une quelconque des revendications 7 à 10, où le composé ester polyfonctionnel est un composé représenté par la formule (I) : où R¹, R², R³ et R⁴ sont indépendamment un radical alkyle ou un radical phényle, et le nombre d'atomes de carbone du radical alkyle ou du radical phényle se situe dans l'intervalle allant de 10 à 30, et il est de préférence le tétrastéarate de pentaérythritol ou le tétramyristate de pentaérythritol.

12. Procédé de production selon l'une quelconque des revendications 7 à 11, où la composition de monomère polymérisable comprend en outre un monomère de réticulation.

13. Procédé de production selon l'une quelconque des revendications 7 à 12, où l'initiateur de polymérisation radicalaire oléo-soluble est un peroxyde organique dont la température de 10 heures de demi-vie se situe dans l'intervalle allant de 60 à 80°C, et dont le poids moléculaire est de 250 ou moins.

14. Procédé de production selon l'une quelconque des revendications 7 à 13, où dans l'étape (1), la polymérisation en suspension est réalisée dans un milieu aqueux de dispersion contenant un colloïde d'un hydroxyde métallique difficilement hydrosoluble comme agent de dispersion.

15. Procédé de production selon la revendication 14, où le colloïde de l'hydroxyde métallique difficilement hydrosoluble est tel que la valeur cumulative à 50% (D₅₀) de sa distribution du diamètre particulaire en nombre est d'au plus 0,5 µm, et que la valeur cumulative à 90% (D₉₀) de sa distribution du diamètre particulaire en nombre est d'au plus 1 µm.

16. Procédé de production selon la revendication 14, où le colloïde de l'hydroxyde métallique difficilement hydrosoluble est obtenu en ajustant le pH d'une solution aqueuse d'un composé métallique polyvalent hydrosoluble à 7 ou plus.

17. Procédé de production selon la revendication 15, où le colloïde de l'hydroxyde métallique difficilement hydrosoluble est obtenu par réaction d'un composé métallique polyvalent hydrosoluble avec un hydroxyde de métal alcalin en phase aqueuse.

18. Procédé de production selon la revendication 7, où dans l'étape (1), un mélange liquide contenant au moins le composé ester polyfonctionnel, le colorant, le monomère polymérisable pour le coeur et un initiateur de polymérisation radicalaire est préparé, le mélange liquide est versé dans le milieu aqueux de dispersion contenant l'agent de dispersion pour former de minuscules gouttelettes sous agitation, et la polymérisation en suspension est alors effectuée à une température allant de 30 à 200°C.

19. Procédé de production selon l'une quelconque des revendications 7 à 18, où dans l'étape (1), les particules de coeur composées des particules polymères colorées ayant un diamètre particulaire moyen en volume (dv) allant de 0,5 à 20 µm et un rapport (dv/dp) du diamètre particulaire moyen en volume (dv) au diamètre particulaire moyen en nombre (dp) d'au plus 1,7 sont préparées.

20. Procédé de production selon l'une quelconque des revendications 7 à 19, où dans l'étape (2), le monomère polymérisable pour la coque est préparé en gouttelettes ayant un diamètre moyen en nombre des gouttelettes inférieur à celui des particules de coeur, puis en soumettant à la polymérisation en suspension.

21. Procédé de production selon l'une quelconque des revendications 7 à 20, où le monomère polymérisable pour la coque est un monomère ayant une solubilité d'au moins 0,1% en poids dans l'eau à 20°C.

22. Procédé de production selon l'une quelconque des revendications 7 à 20, où le monomère polymérisable pour la coque est un monomère ayant une solubilité inférieure à 0,1% en poids dans l'eau à 20°C, et dans l'étape (2), ledit monomère polymérisable pour la coque et un solvant organique ayant une solubilité d'au moins 5% en poids dans l'eau à 20°C sont ajoutés pour réaliser la polymérisation en suspension.

23. Procédé de production selon l'une quelconque des revendications 7 à 22, où dans l'étape (2), le monomère polymérisable pour la coque et un agent du contrôle de la charge sont ajoutés pour réaliser la polymérisation en suspension.

24. Procédé de production selon l'une quelconque des revendications 7 à 23, où dans l'étape (2), la coque constituée d'une couche polymère ayant une épaisseur moyenne de film allant de 0,001 à 1 µm est formée.

25. Procédé de formation d'image, comprenant les étapes d'application d'un toner sur la surface d'un élément photosensible, sur lequel une image latente électrostatique a été formée, pour rendre visible l'image latente, puis de transfert de l'image visible sur un milieu de transfert, où le toner est un toner polymérisé tel que défini dans l'une quelconque des revendications 1 à 6.

26. Utilisation d'un toner polymérisé tel que défini dans l'une quelconque des revendications 1 à 6, dans un appareil de formation d'image, comprenant un élément photosensible, un moyen pour charger la surface de l'élément photosensible, un moyen pour former une image latente électrostatique sur la surface de l'élément photosensible, un moyen pour réceptionner un toner, un moyen pour fournir le toner pour développer l'image latente électrostatique sur la surface de l'élément photosensible, ce qui forme une image de toner, et un moyen pour transférer l'image de toner depuis la surface de l'élément photosensible sur un milieu de transfert.
